



US010538719B2

(12) **United States Patent**  
Sivik et al.

(10) **Patent No.:** US 10,538,719 B2  
(45) **Date of Patent:** Jan. 21, 2020

(54) **TREATMENT COMPOSITIONS**

- (71) Applicant: **The Procter & Gamble Company**, Cincinnati, OH (US)
- (72) Inventors: **Mark Robert Sivik**, Mason, OH (US); **Travis Kyle Hodgdon**, Cincinnati, OH (US); **Alessandro Corona, III**, Mason, OH (US); **Robert Richard Dykstra**, West Chester, OH (US); **Richard Timothy Hartshorn**, Lawrenceburg, IN (US); **Nicholas David Vetter**, Cleves, OH (US); **Tessa Xuan**, Cincinnati, OH (US)
- (73) Assignee: **The Procter & Gamble Company**, Cincinnati, OH (US)
- (\*) Notice: Subject to any disclaimer, the term of this patent is extended or adjusted under 35 U.S.C. 154(b) by 622 days.

(21) Appl. No.: 14/806,696

(22) Filed: Jul. 23, 2015

(65) **Prior Publication Data**

US 2016/0024434 A1 Jan. 28, 2016

**Related U.S. Application Data**

(60) Provisional application No. 62/027,879, filed on Jul. 23, 2014, provisional application No. 62/083,938, filed on Nov. 25, 2014.

- (51) **Int. Cl.**  
**CIID 3/00** (2006.01)  
**CIID 3/30** (2006.01)  
**CIID 3/34** (2006.01)  
**CIID 3/37** (2006.01)  
**CIID 3/50** (2006.01)

- (52) **U.S. Cl.**  
CPC ..... **CIID 3/001** (2013.01); **CIID 3/30** (2013.01); **CIID 3/349** (2013.01); **CIID 3/373** (2013.01); **CIID 3/3769** (2013.01); **CIID 3/505** (2013.01)

- (58) **Field of Classification Search**  
CPC ..... C11D 3/001  
See application file for complete search history.

(56) **References Cited**

## U.S. PATENT DOCUMENTS

- 4,137,180 A 1/1979 Naik et al.  
4,199,464 A 4/1980 Cambre  
4,528,321 A 7/1985 Allen et al.  
5,296,622 A 3/1994 Uphues et al.  
5,759,990 A 6/1998 Wahl et al.  
6,271,192 B1 8/2001 Verstrat et al.  
6,326,430 B1 12/2001 Berte  
6,348,541 B1 2/2002 Kanda et al.  
6,361,781 B2 3/2002 Lorant  
6,376,456 B1 4/2002 Murphy et al.  
6,413,920 B1 7/2002 Bettoli et al.  
6,494,920 B1 12/2002 Weuthen et al.

|                  |         |                                     |
|------------------|---------|-------------------------------------|
| 6,620,777 B2     | 9/2003  | Heibel et al.                       |
| 6,924,261 B2     | 8/2005  | Grandmaire et al.                   |
| 6,992,058 B2     | 1/2006  | Grandmaire et al.                   |
| 7,063,895 B2     | 6/2006  | Rodrigues et al.                    |
| 7,378,033 B2     | 5/2008  | Harrison et al.                     |
| 7,381,417 B2     | 6/2008  | Gamez-Garcia                        |
| 7,981,850 B2     | 7/2011  | Doi et al.                          |
| 8,188,022 B2     | 5/2012  | Sengupta et al.                     |
| 8,211,414 B2     | 7/2012  | Chen et al.                         |
| 8,524,649 B2     | 9/2013  | Leyrer et al.                       |
| 8,563,498 B2     | 10/2013 | Gizaw et al.                        |
| 8,741,831 B2     | 6/2014  | Jaynes et al.                       |
| 8,835,373 B2     | 9/2014  | Miravet Celades et al.              |
| 9,018,154 B2     | 4/2015  | Blondel                             |
| 9,441,188 B2     | 9/2016  | Schramm, Jr. et al.                 |
| 2002/0132749 A1* | 9/2002  | Smith ..... C11D 1/62<br>510/327    |
| 2004/0038851 A1  | 2/2004  | Aubay et al.                        |
| 2004/0065208 A1  | 4/2004  | Hart et al.                         |
| 2004/0071716 A1  | 4/2004  | Jansen et al.                       |
| 2004/0116321 A1* | 6/2004  | Salesses ..... C11D 1/62<br>510/515 |
| 2004/0116322 A1  | 6/2004  | Yianakopoulos et al.                |
| 2004/0204337 A1  | 10/2004 | Corona, III et al.                  |
| 2004/0229769 A1  | 11/2004 | Smith et al.                        |
| 2005/0003980 A1  | 1/2005  | Baker et al.                        |
| 2005/0245668 A1  | 11/2005 | Green et al.                        |
| 2005/0256027 A1* | 11/2005 | Heibel ..... C11D 1/40<br>510/515   |
| 2006/0094639 A1  | 5/2006  | Martin et al.                       |

(Continued)

## FOREIGN PATENT DOCUMENTS

|    |              |         |                  |
|----|--------------|---------|------------------|
| CA | 2482306 A1 * | 3/2003  | ..... A01N 33/12 |
| CA | 2482306 C    | 10/2011 | (Continued)      |

## OTHER PUBLICATIONS

International Preliminary Report on Patentability; International Application No. PCT/US2015/041654; dated Nov. 3, 2016; 12 pages.  
U.S. Appl. No. 14/806,680, filed Jul. 23, 2015, Sivik, et al.  
U.S. Appl. No. 14/806,682, filed Jul. 23, 2015, Dykstra, et al.  
U.S. Appl. No. 14/806,684, filed Jul. 23, 2015, Dykstra, et al.  
U.S. Appl. No. 14/806,685, filed Jul. 23, 2015, Dykstra, et al.  
U.S. Appl. No. 14/806,688, filed Jul. 23, 2015, Dykstra, et al.  
U.S. Appl. No. 14/806,690, filed Jul. 23, 2015, Sivik, et al.  
U.S. Appl. No. 14/806,691, filed Jul. 23, 2015, Sivik, et al.  
U.S. Appl. No. 14/806,692, filed Jul. 23, 2015, Sivik, et al.  
U.S. Appl. No. 14/806,694, filed Jul. 23, 2015, Sivik, et al.  
Invitation to pay additional fees; International Application No. PCT/US2015/041654; dated Nov. 2, 2015; 6 pages.

(Continued)

Primary Examiner — Mark Eashoo

Assistant Examiner — M. Reza Asdjodi

(74) Attorney, Agent, or Firm — Gregory S. Darley-Emerson

(57) **ABSTRACT**

The present invention relates to treatment compositions containing polymer systems that provide stability and benefit agent deposition as well as methods of making and using same. Such treatment compositions may be used for example as through the wash and/or through the rinse fabric enhancers as well as unit dose treatment compositions.

**18 Claims, No Drawings**

| (56)                  | References Cited |                           |             |    |                    |         |                   |
|-----------------------|------------------|---------------------------|-------------|----|--------------------|---------|-------------------|
| U.S. PATENT DOCUMENTS |                  |                           |             |    |                    |         |                   |
| 2006/0252669 A1*      | 11/2006          | Heibel .....              | C11D 1/40   | EP | 1 352 948 A1       | 10/2003 |                   |
|                       |                  | 510/515                   |             | EP | 1 625 195 B1       | 5/2007  |                   |
| 2007/0099817 A1*      | 5/2007           | Smith .....               | C11D 1/62   | EP | 1 740 682 B1       | 6/2009  |                   |
|                       |                  | 510/515                   |             | EP | 1 756 168 B1       | 7/2009  |                   |
| 2007/0275866 A1       | 11/2007          | Dykstra                   |             | EP | 2 284 250 A1       | 2/2011  |                   |
| 2007/0293413 A1       | 12/2007          | McFarland et al.          |             | EP | 1 781 717 B1       | 11/2012 |                   |
| 2008/0076692 A1       | 3/2008           | Carvell et al.            |             | FR | 2862975 B1         | 2/2006  |                   |
| 2008/0167453 A1*      | 7/2008           | Goettel .....             | A61K 8/416  | GB | 2 002 400 A        | 2/1979  |                   |
|                       |                  | 534/560                   |             | JP | 2012154010 A       | 8/2012  |                   |
| 2008/0295256 A1       | 12/2008          | Broze et al.              |             | JP | 2012158547 A       | 8/2012  |                   |
| 2008/0312343 A1       | 12/2008          | Braun et al.              |             | JP | 5034078 B2         | 9/2012  |                   |
| 2009/0062174 A1       | 3/2009           | Green et al.              |             | JP | 5528660 B2         | 6/2014  |                   |
| 2010/0035791 A1       | 2/2010           | Igarashi et al.           |             | KR | 20150100549 A      | 9/2015  |                   |
| 2010/0190679 A1       | 7/2010           | Vanpachtenbeke et al.     |             | WO | WO 96/07689 A1     | 3/1996  |                   |
| 2011/0245141 A1       | 10/2011          | Gizaw et al.              |             | WO | WO 99/20725 A1     | 4/1999  |                   |
| 2011/0245142 A1       | 10/2011          | Gizaw et al.              |             | WO | WO 02/057400 A2    | 7/2002  |                   |
| 2011/0269663 A1*      | 11/2011          | Clowes .....              | C11D 1/62   | WO | WO 03/002699 A1    | 1/2003  |                   |
|                       |                  | 510/515                   |             | WO | WO 03/102043 A1    | 12/2003 |                   |
| 2011/0301312 A1       | 12/2011          | Blondel                   |             | WO | WO 2004/050812 A1  | 6/2004  |                   |
| 2012/0142578 A1*      | 6/2012           | Panandiker .....          | C11D 1/667  | WO | WO 2004/061065 A1  | 7/2004  |                   |
|                       |                  | 510/515                   |             | WO | WO 2005/087907 A1  | 9/2005  |                   |
| 2013/0065813 A1       | 3/2013           | Miravet Celades et al.    |             | WO | WO 2005087907 A1 * | 9/2005  | ..... C11D 3/3723 |
| 2013/0109612 A1       | 5/2013           | Corona, III et al.        |             | WO | WO 2005/097834 A2  | 10/2005 |                   |
| 2013/0121944 A1*      | 5/2013           | Leyrer .....              | C11D 3/3765 | WO | WO 2005/103215 A1  | 11/2005 |                   |
|                       |                  | 424/70.16                 |             | WO | WO 2008/005693 A2  | 1/2008  |                   |
| 2013/0121945 A1       | 5/2013           | Leyrer et al.             |             | WO | WO 2008005693 A2 * | 1/2008  | ..... C11D 3/37   |
| 2013/0129657 A1       | 5/2013           | Streuli                   |             | WO | WO 2010/078959 A1  | 7/2010  |                   |
| 2013/0197101 A1       | 8/2013           | Braun et al.              |             | WO | WO 2010/079100 A1  | 7/2010  |                   |
| 2013/0310300 A1       | 11/2013          | Leyrer et al.             |             | WO | WO 2010079100 A1 * | 7/2010  | ..... C11D 1/62   |
| 2013/0310301 A1*      | 11/2013          | Sivik .....               | C11D 1/62   | WO | WO 2012/076432 A1  | 6/2012  |                   |
|                       |                  | 510/516                   |             | WO | WO 2013/068388 A1  | 5/2013  |                   |
| 2014/0047649 A1       | 2/2014           | Blondel                   |             | WO | WO 2013/068394 A1  | 5/2013  |                   |
| 2014/0315779 A1       | 10/2014          | Zander                    |             | WO | WO 2013/142486 A1  | 9/2013  |                   |
| 2014/0378639 A1       | 12/2014          | Blondel et al.            |             | WO | WO 2013/189010 A1  | 12/2013 |                   |
| 2015/0191677 A1       | 7/2015           | Blondel                   |             | WO | WO 2015/130088 A1  | 9/2015  |                   |
| 2015/0197708 A1       | 7/2015           | Jin                       |             |    |                    |         |                   |
| 2015/0329799 A1       | 11/2015          | Schramm, Jr. et al.       |             |    |                    |         |                   |
| 2015/0337239 A1       | 11/2015          | Gonzalez de Cossio et al. |             |    |                    |         |                   |
| 2016/0024426 A1       | 1/2016           | Sivik et al.              |             |    |                    |         |                   |
| 2016/0024427 A1*      | 1/2016           | Sivik .....               | C11D 1/62   |    |                    |         |                   |
|                       |                  | 8/137                     |             |    |                    |         |                   |
| 2016/0024428 A1       | 1/2016           | Dykstra et al.            |             |    |                    |         |                   |
| 2016/0024429 A1       | 1/2016           | Dykstra et al.            |             |    |                    |         |                   |
| 2016/0024430 A1       | 1/2016           | Dykstra et al.            |             |    |                    |         |                   |
| 2016/0024431 A1       | 1/2016           | Dykstra et al.            |             |    |                    |         |                   |
| 2016/0024432 A1       | 1/2016           | Sivik et al.              |             |    |                    |         |                   |
| 2016/0024433 A1       | 1/2016           | Sivik et al.              |             |    |                    |         |                   |
| 2016/0032220 A1*      | 2/2016           | Sivik .....               | C11D 3/001  |    |                    |         |                   |
|                       |                  | 510/515                   |             |    |                    |         |                   |
| 2017/0191002 A1       | 7/2017           | Dykstra et al.            |             |    |                    |         |                   |
| 2017/0247637 A1       | 8/2017           | Dykstra et al.            |             |    |                    |         |                   |
| 2017/0298295 A1       | 10/2017          | Dykstra et al.            |             |    |                    |         |                   |
| 2017/0342345 A1       | 11/2017          | Sivik et al.              |             |    |                    |         |                   |

## FOREIGN PATENT DOCUMENTS

|    |              |         |
|----|--------------|---------|
| CN | 101724132 B  | 11/2011 |
| EP | 0 172 025 A2 | 2/1986  |
| EP | 0 172 723 A2 | 2/1986  |
| EP | 0 172 724 A2 | 2/1986  |
| EP | 0 343 840 A2 | 11/1989 |

## OTHER PUBLICATIONS

International Search Report; International Application No. PCT/US2015/041656; dated Oct. 9, 2015; 10 pages.  
 International Search Report; International Application No. PCT/US2015/041657; dated Oct. 8, 2015; 11 pages.  
 International Search Report; International Application No. PCT/US2015/041658; dated Oct. 8, 2015; 11 pages.  
 International Search Report; International Application No. PCT/US2015/041659; dated Nov. 2, 2015; 15 pages.  
 International Search Report; International Application No. PCT/US2015/041737; dated Oct. 23, 2015; 10 pages.  
 International Search Report; International Application No. PCT/US2015/041741; dated Oct. 8, 2015; 11 pages.  
 International Search Report; International Application No. PCT/US2015/041640; dated Oct. 8, 2015; 11 pages.  
 International Search Report; International Application No. PCT/US2015/041641; dated Oct. 13, 2015; 10 pages.  
 International Search Report; International Application No. PCT/US2015/041642; dated Oct. 8, 2015; 11 pages.  
 Schuck, Peter, Size-Distribution Analysis of Macromolecules by Sedimentation Velocity Ultracentrifugation and Lamm Equation Modeling, Biophysical Journal, Mar. 2000, pp. 1606-1619, vol. 78, No. 3.  
 ASTM D3954-94 (Reapproved 2010), Standard Test Method for Dropping Point of Waxes.

\* cited by examiner

## 1

## TREATMENT COMPOSITIONS

## FIELD OF THE INVENTION

The present invention relates to treatment compositions and processes of making and using same.

## BACKGROUND OF THE INVENTION

Treatment compositions, such as fabric treatment compositions, typically comprise benefit agents such as silicones, fabric softener actives, perfumes and perfume microcapsules. Generally there are trade-offs associated with using multiple benefit agents in one treatment composition. Such trade-offs include instability, as well as the loss or reduction of one or more of the benefit agents' benefits. A reduction in one of the benefit agent's levels can improve the performance of another benefit agent, yet the performance of the benefit agent that is being reduced suffers. In an effort to solve this dilemma, industry has turned to polymers. Current polymers systems can improve a treatment composition's stability but such improvement in stability comes with a decrease in freshness.

Applicants recognized that the traditional polymer system architecture was the source of the stability and freshness problems. Applicants recognized that, for fabric softeners, in particular low pH fabric softeners, the judicious selection of at least two polymers, one synthetic and one derived from saccharides, the fabric softener active can be reduced so that the active does not decrease perfume effectiveness and yet, surprisingly, the feel benefit and stability are maintained. While not being bound by theory, Applicants believe that the proper selection of such polymers increases active hydration which promotes diffusion of benefit agents such as perfumes, and leads to more efficient softener active performance.

## SUMMARY OF THE INVENTION

The present invention relates to treatment compositions containing polymer systems that provide stability and benefit agent deposition as well as methods of making and using same. Such treatment compositions may be used for example as through the wash and/or through the rinse fabric enhancers as well as unit dose treatment compositions.

## DETAILED DESCRIPTION OF THE INVENTION

## Definitions

As used herein, the term "fabric and home care product" is a subset of cleaning and treatment compositions that includes, unless otherwise indicated, granular or powder-form all-purpose or "heavy-duty" washing agents, especially cleaning detergents; liquid, gel or paste-form all-purpose washing agents, especially the so-called heavy-duty liquid types; liquid fine-fabric detergents; hand dishwashing agents or light duty dishwashing agents, especially those of the high-foaming type; machine dishwashing agents, including the various tablet, granular, liquid and rinse-aid types for household and institutional use; liquid cleaning and disinfecting agents, including antibacterial hand-wash types, cleaning bars, car or carpet shampoos, bathroom cleaners including toilet bowl cleaners; and metal cleaners, fabric conditioning products including softening and/or freshening that may be in liquid, solid and/or dryer sheet form; as well

## 2

as cleaning auxiliaries such as bleach additives and "stain-stick" or pre-treat types, substrate-laden products such as dryer added sheets, dry and wetted wipes and pads, nonwoven substrates, and sponges; as well as sprays and mists. All of such products which are applicable may be in standard, concentrated or even highly concentrated form even to the extent that such products may in certain aspect be non-aqueous.

As used herein, the term "situs" includes paper products, fabrics, garments and hard surfaces.

As used herein, articles such as "a", "an", and "the" when used in a claim, are understood to mean one or more of what is claimed or described.

Unless otherwise noted, all component or composition levels are in reference to the active level of that component or composition, and are exclusive of impurities, for example, residual solvents or by-products, which may be present in commercially available sources.

All percentages and ratios are calculated by weight unless otherwise indicated. All percentages and ratios are calculated based on the total composition unless otherwise indicated.

It should be understood that every maximum numerical limitation given throughout this specification includes every lower numerical limitation, as if such lower numerical limitations were expressly written herein. Every minimum numerical limitation given throughout this specification will include every higher numerical limitation, as if such higher numerical limitations were expressly written herein. Every numerical range given throughout this specification will include every narrower numerical range that falls within such broader numerical range, as if such narrower numerical ranges were all expressly written herein.

## Fabric Treatment Compositions

A composition comprising, based upon total composition weight:

a) from about 0.01% to about 5%, preferably from about 0.02% to about 3.5%, more preferably from about 0.05% to about 2.5% of a polymeric mixture that comprises:

(i) polymer system 1 that comprises a first polymer being derived from saccharides, preferably said first polymer that is derived from saccharides is hydrophobically, hydrophilically, and/or cationically modified, or a polymer system 1 that comprises a first polymer being derived from saccharides, preferably said first polymer that is derived from saccharides is hydrophobically, and/or cationically modified, and a second polymer being derived from the polymerization of from about 5 to 100 mole percent of a cationic vinyl addition monomer, from about 0 to 95 mole percent of a non-ionic vinyl addition monomer, from about 0 to about 50 mole percent, preferably 1 to 25 mole percent of an anionic monomer, from about 0 ppm to 45 ppm of a cross-linking agent comprising two or more ethylenic functions, 0 ppm to about 10,000 ppm chain transfer agent, preferably 5 ppm to 5,000 ppm, more preferably 50 to 1,000 ppm chain transfer agent, preferably said second polymer has a viscosity slope <3.7; in one aspect said second polymer is a linear or branched, uncross-linked polyethyleneimine, preferably said polyethyleneimine is branched and uncross-linked; or

(ii) polymer system 2 that comprises a first polymer and a second polymer, preferably said first polymer and said second polymer being present in a ratio of about

- 1:5 to about 10:1, preferably, about 1:2 to about 5:1, most preferably about 1:1 to about 3:1; said first polymer is derived from the polymerization of from about 5 to 100 mole percent of a cationic vinyl addition monomer, from about 0 to 95 mole percent of a non-ionic vinyl addition monomer, from about 0 to about 50 mole percent, preferably 1 to 25 mole percent of an anionic monomer, from about 50 ppm to 1,950 ppm of a cross-linking agent comprising two or more ethylenic functions, 0 ppm to about 10,000 ppm chain transfer agent, preferably 5 ppm to 5,000 ppm, more preferably 50 to 1,000 ppm chain transfer agent, preferably said first polymer has a viscosity slope  $>3.7$ ; said second polymer being derived from saccharides, preferably said first polymer that is derived from saccharides is hydrophobically, hydrophilically, and/or cationically modified; and
- b) from about 0% to about 35%, preferably from about 1% to about 35%, more preferably from about 2% to about 25%, more preferably from about 3% to about 20%, more preferably from about 5% to about 15%, most preferably from about 8% to about 12% of a fabric softener active said composition being a fabric and home care product is disclosed.

In one aspect of said composition:

- a) for polymer system 1 said first polymer is derived from guar, cellulose, starch, chitosan, cassia, hyaluronan, konjac glucomannan, xyloglucan, kappa-carrageenan, gellan gum, succinoglycan, xanthan, curdlan and schizophyllan; preferably said first polymer is derived from guar, cellulose, starch, chitosan, cassia, hyaluronan, konjac glucomannan, xyloglucan, kappa-carrageenan, gellan gum, succinoglycan, xanthan, curdlan and schizophyllan is hydrophobically, hydrophilically, and/or cationically modified; and said second polymer is derived from the polymerization of from about 10 to 95 mole percent of a cationic vinyl addition monomer, preferably 20 mole percent to 90 mole percent from about 5 to 90 mole percent of a non-ionic vinyl addition monomer, preferably 10 to 80 mole percent, from about 0 ppm to 40 ppm of a cross-linking agent comprising two or more ethylenic functions, preferably 0 ppm to 20 ppm, 0 ppm to about 10,000 ppm chain transfer agent, preferably said second polymer has a viscosity slope  $<3.7$ ;
- b) for polymer system 2 said first polymer is derived from the polymerization of from about 10 to 95 mole percent of a cationic vinyl addition monomer, preferably 20 mole percent to 90 mole percent from about 5 to 90 mole percent of a non-ionic vinyl addition monomer, preferably 10 mole percent to 80 mole percent from about 60 ppm to 1,900 ppm of a cross-linking agent comprising two or more ethylenic functions, preferably 75 to 1,800 ppm to about 10,000 ppm chain transfer agent, preferably said first polymer has a viscosity slope  $>3.7$ , with the proviso that said first polymer does not comprise an acrylamide unit; and said second polymer is derived from starch, cellulose, and guar; preferably said first polymer is derived from starch, cellulose, and guar that is hydrophobically, hydrophilically, and/or cationically modified.

In one aspect of said composition, said polymer being derived from saccharides are catatonically modified and have a cationic charge density ranging from about 0.2 meq/gm to about 5 meq/gm, preferably at least about 0.4 meq/gm, more preferably at least about 0.6 meq/gm, but also

preferably less than about 3 meq/gm, more preferably less than about 2 meq/gm, at the pH of intended use of the fabric softening composition.

In one aspect of said composition, said fabric softener active is selected from the group consisting of a quaternary ammonium compound, a silicone polymer, a polysaccharide, a clay, an amine, a fatty ester, a dispersible polyolefin, a polymer latex and mixtures thereof.

In one aspect of said composition:

- a) said quaternary ammonium compound comprises an alkyl quaternary ammonium compound, preferably said alkyl quaternary ammonium compound is selected from the group consisting of a monoalkyl quaternary ammonium compound, a dialkyl quaternary ammonium compound, a trialkyl quaternary ammonium compound and mixtures thereof;
- b) said silicone polymer is selected from the group consisting of cyclic silicones, polydimethylsiloxanes, aminosilicones, cationic silicones, silicone polyethers, silicone resins, silicone urethanes, and mixtures thereof;
- c) said clay comprises a smectite clay;
- d) said dispersible polyolefin is selected from the group consisting of polyethylene, polypropylene and mixtures thereof; and
- e) said fatty ester is selected from the group consisting of a polyglycerol ester, a sucrose ester, a glycerol ester and mixtures thereof.

In one aspect of said composition said fabric softener active comprises a material selected from the group consisting of monoesterquats, diesterquats, triesterquats, and mixtures thereof. Preferably, said monoesterquats and diesterquats are selected from the group consisting of bis-(2-hydroxypropyl)-dimethylammonium methylsulfate fatty acid ester and isomers of bis-(2-hydroxypropyl)-dimethylammonium methylsulfate fatty acid ester and/or mixtures thereof, 1,2-di(acyloxy)-3-trimethylammoniopropane chloride, N, N-bis(stearoyl-oxy-ethyl)-N,N-dimethyl ammonium chloride, N,N-bis(tallowoyl-oxy-ethyl) N,N-dimethyl ammonium chloride, N,N-bis(stearoyl-oxy-ethyl)-N-(2 hydroxyethyl)-N-methyl ammonium methylsulfate, N,N-bis-(stearyl-2-hydroxypropyl)-N,N-dimethylammonium methylsulfate, N,N-bis(tallowoyl-2-hydroxypropyl)-N,N-dimethylammonium methylsulfate, N,N-bis-(palmitoyl-2-hydroxypropyl)-N,N-dimethylammonium methylsulfate, N,N-bis-(stearyl-2-hydroxypropyl)-N,N-dimethylammonium chloride, 1,2-di-(stearyl-oxy)-3-trimethyl ammoniumpropane chloride, dicanoladimethylammonium chloride, di(hard)tallowdimethylammonium chloride, dicanoladimethylammonium methylsulfate, 1-methyl-1-stearylamo-ethyl-2-stearylimidazolinium methylsulfate, 1-tallowylamidoethyl-2-tallowylimidazoline, dipalmylmethyl hydroxyethylammonium methylsulfate and mixtures thereof.

In one aspect of said composition said, fabric softening active has an Iodine Value of between 0-140, preferably 5-100, more preferably 10-80, even more preferably 15-70, even more preferably 18-60, most preferably 18-25. When partially hydrogenated fatty acid quaternary ammonium compound softener is used, the most preferable range is 25-60.

In one aspect of said composition, said composition comprises a quaternary ammonium compound and a silicone polymer, preferably from about 0.001% to about 10%, from about 0.1% to about 8%, more preferably from about 0.5% to about 5%, of said silicone polymer.

In one aspect of said composition, said composition comprises, in addition to said fabric softener active, from about 0.001% to about 5%, preferably from about 0.1% to about 3%, more preferably from about 0.2% to about 2% of a stabilizer that comprises a alkyl quaternary ammonium compound, preferably said alkyl quaternary ammonium compound comprises a material selected from the group consisting of a monoalkyl quaternary ammonium compound, a dialkyl quaternary ammonium compound, a trialkyl quaternary ammonium compound and mixtures thereof, more preferably said alkyl quaternary ammonium compound comprises a monoalkyl quaternary ammonium compound and/or di-alkyl quaternary ammonium compound.

In one aspect of said composition, said synthetic polymer is derived from

- a.) a monomer selected from the group consisting of  
(i) a cationic monomer according to formula (I):



wherein:

- R<sub>1</sub> is chosen from hydrogen, or C<sub>1</sub>-C<sub>4</sub> alkyl;  
R<sub>2</sub> is chosen from hydrogen or methyl;  
R<sub>3</sub> is chosen from C<sub>1</sub>-C<sub>4</sub> alkylene;  
R<sub>4</sub>, R<sub>5</sub>, and R<sub>6</sub> are each independently chosen from hydrogen, C<sub>1</sub>-C<sub>4</sub> alkyl, C<sub>1</sub>-C<sub>4</sub> alkyl alcohol or C<sub>1</sub>-C<sub>4</sub> alkoxy;  
X is chosen from —O—, or —NH—; and  
Y is chosen from Cl, Br, I, hydrogensulfate or methylsulfate,

- (ii) a non-ionic monomer having formula (II)



wherein:

- R<sub>7</sub> is chosen from hydrogen or C<sub>1</sub>-C<sub>4</sub> alkyl;  
R<sub>8</sub> is chosen from hydrogen or methyl;  
R<sub>9</sub> and R<sub>10</sub> are each independently chosen from hydrogen, C<sub>1</sub>-C<sub>30</sub> alkyl, C<sub>1</sub>-C<sub>4</sub> alkyl alcohol or C<sub>1</sub>-C<sub>4</sub> alkoxy,

- (iii) an anionic monomer selected from the group consisting of acrylic acid, methacrylic acid, itaconic acid, crotonic acid, maleic acid, fumaric acid, as well as monomers performing a sulfonic acid or phosphonic acid functions, such as 2-acrylamido-2-methyl propane sulfonic acid, and their salts.

- b.) wherein said cross-linking agent is selected from the group consisting of 1,2,4-trivinylcyclohexane 1,7-octadiene, allyl acrylates and methacrylates, allyl-acrylamides and allyl-methacrylamides, allyl-acrylamides and allyl-methacrylamides, bisacrylamidoacetic acid, bisacrylamidoacetic acid, butadiene diacrylates and dimethacrylates of glycols and polyglycols, N,N'-methylen-bisacrylamide and polyol polyallyl ethers, such as polyallylsaccharose and pentaerythrol triallylether,

tetra allyl ammonium chloride, di(ethylene glycol) diacrylate, di(ethylene glycol) dimethacrylate, divinyl benzene, ethylene glycol diacrylate, ethylene glycol dimethacrylate, N,N'-(1,2-dihydroxyethylene)bisacrylamide, tetra(ethylene glycol) diacrylate, tri(ethylene glycol) dimethacrylate and mixtures thereof.

- c.) wherein said chain transfer agent is selected from the group consisting of mercaptanes, malic acid, lactic acid, formic acid, isopropanol and hypophosphites, and mixtures thereof.

In one aspect of said composition said cationic monomers are selected from the group consisting of methyl chloride quaternized dimethyl aminoethylammonium acrylate, methyl chloride quaternized dimethyl aminoethylammonium methacrylate and mixtures thereof, and the non-ionic monomers are selected from the group consisting of acrylamide, dimethyl acrylamide and mixtures thereof.

In one aspect of said composition, said composition has a Brookfield viscosity of from about 20 cps to about 1,000 cps, preferably from 30 cps to about 500 cps, and most preferably 40 cps to about 300 cps.

In one aspect of said composition, said composition comprising an adjunct material selected from the group consisting of surfactants, builders, chelating agents, dye transfer inhibiting agents, dispersants, enzymes, and enzyme stabilizers, catalytic materials, bleach activators, hydrogen peroxide, sources of hydrogen peroxide, preformed peracids, polymeric dispersing agents, clay soil removal/anti-redeposition agents, brighteners, suds suppressors, dyes, hueing dyes, perfumes, perfume delivery systems, structure elasticizing agents, carriers, structurants, hydrotropes, processing aids, solvents and/or pigments and mixtures thereof.

In one aspect of said composition, said composition comprises perfume and/or a perfume delivery system, preferably said perfume delivery system comprises perfume microcapsules, preferably said perfume microcapsules comprises a cationic coating.

In one aspect of said composition, said composition comprising one or more types of perfume microcapsules.

In one aspect of said composition, said composition has a pH from about 2 to about 4, preferably from about 2.4 to about 3.6.

In one aspect the viscosity slope of any of the embodiments of Applicants' compositions that are claimed and/or disclosed is determined using Viscosity Slope Method 1, preferably viscosity slope of any of the embodiments of Applicants' compositions that are claimed and/or disclosed is determined using Viscosity Slope Method 2.

When a polymer is described as being hydrophobically modified, suitable methods for achieving a hydrophobic modification include, but are not limited to, C<sub>1</sub>-C<sub>22</sub> alkyl substitution, C<sub>3</sub>-C<sub>12</sub> alkoxylation, and mixtures thereof. When a polymer is described as hydrophilically modified, suitable methods for hydrophytic modification include, but are not limited to, ethoxylation, propoxylation, carboxymethylation, sulfation, sulfonation, oxidation, and mixtures thereof. When a polymer is described as being cationically modified, suitable methods for achieving a cationic modification include, but are not limited to, quaternization, alkylation containing a cationic moiety, protonatable amines, and mixtures thereof.

#### Suitable Fabric Softening Actives

The fluid fabric enhancer compositions disclosed herein comprise a fabric softening active ("FSA"). Suitable fabric softening actives, include, but are not limited to, materials selected from the group consisting of quaternary ammonium compounds, amines, fatty esters, sucrose esters, silicones,

dispersible polyolefins, clays, polysaccharides, fatty acids, softening oils, polymer latexes and mixtures thereof.

Non-limiting examples of water insoluble fabric care benefit agents include dispersible polyethylene and polymer latexes. These agents can be in the form of emulsions, latexes, dispersions, suspensions, and the like. In one aspect, they are in the form of an emulsion or a latex. Dispersible polyethylenes and polymer latexes can have a wide range of particle size diameters ( $\chi_{50}$ ) including but not limited to from about 1 nm to about 100  $\mu\text{m}$ ; alternatively from about 10 nm to about 10  $\mu\text{m}$ . As such, the particle sizes of dispersible polyethylenes and polymer latexes are generally, but without limitation, smaller than silicones or other fatty oils.

Generally, any surfactant suitable for making polymer emulsions or emulsion polymerizations of polymer latexes can be used to make the water insoluble fabric care benefit agents of the present invention. Suitable surfactants consist of emulsifiers for polymer emulsions and latexes, dispersing agents for polymer dispersions and suspension agents for polymer suspensions. Suitable surfactants include anionic, cationic, and nonionic surfactants, or combinations thereof. In one aspect, such surfactants are nonionic and/or anionic surfactants. In one aspect, the ratio of surfactant to polymer in the water insoluble fabric care benefit agent is about 1:100 to about 1:2; alternatively from about 1:50 to about 1:5, respectively. Suitable water insoluble fabric care benefit agents include but are not limited to the examples described below.

Quats—Suitable quats include but are not limited to, materials selected from the group consisting of ester quats, amide quats, imidazoline quats, alkyl quats, amidoester quats and mixtures thereof. Suitable ester quats include but are not limited to, materials selected from the group consisting of monoester quats, diester quats, triester quats and mixtures thereof. In one aspect, a suitable ester quat is bis-(2-hydroxypropyl)-dimethylammonium methylsulfate fatty acid ester having a molar ratio of fatty acid moieties to amine moieties of from 1.85 to 1.99, an average chain length of the fatty acid moieties of from 16 to 18 carbon atoms and an iodine value of the fatty acid moieties, calculated for the free fatty acid, which has an Iodine Value of between 0-140, preferably 5-100, more preferably 10-80, even more preferably 15-70, even more preferably 18-55, most preferably 18-25. When a soft tallow quaternary ammonium compound softener is used, the most preferable range is 25-60. In one aspect, the cis-trans-ratio of double bonds of unsaturated fatty acid moieties of the bis-(2-hydroxypropyl)-dimethylammonium methylsulfate fatty acid ester is from 55:45 to 75:25, respectively. Suitable amide quats include but are not limited to, materials selected from the group consisting of monoamide quats, diamide quats and mixtures thereof. Suitable alkyl quats include but are not limited to, materials selected from the group consisting of mono alkyl quats, dialkyl quats, trialkyl quats, tetraalkyl quats and mixtures thereof.

Amines—Suitable amines include but are not limited to, materials selected from the group consisting of amidoesteramines, amidoamines, imidazoline amines, alkyl amines, amidoester amines and mixtures thereof. Suitable ester amines include but are not limited to, materials selected from the group consisting of monoester amines, diester amines, triester amines and mixtures thereof. Suitable amido quats include but are not limited to, materials selected from the group consisting of monoamido amines, diamido amines and mixtures thereof. Suitable alkyl amines include but are

not limited to, materials selected from the group consisting of mono alkylamines, dialkyl amines quats, trialkyl amines, and mixtures thereof.

In one embodiment, the fabric softening active is a quaternary ammonium compound suitable for softening fabric in a rinse step. In one embodiment, the fabric softening active is formed from a reaction product of a fatty acid and an aminoalcohol obtaining mixtures of mono-, di-, and, in one embodiment, tri-ester compounds. In another embodiment, the fabric softening active comprises one or more softener quaternary ammonium compounds such, but not limited to, as a monoalkyquaternary ammonium compound, dialkylquaternary ammonium compound, a diamido quaternary compound, a diester quaternary ammonium compound, or a combination thereof.

In one aspect, the fabric softening active comprises a diester quaternary ammonium or protonated diester ammonium (hereinafter “DQA”) compound composition. In certain embodiments of the present invention, the DQA compound compositions also encompass diamido fabric softening actives and fabric softening actives with mixed amido and ester linkages as well as the aforementioned diester linkages, all herein referred to as DQA.

In one aspect, said fabric softening active may comprise, as the principal active, compounds of the following formula:



wherein each R comprises either hydrogen, a short chain C<sub>1</sub>-C<sub>6</sub>, in one aspect a C<sub>1</sub>-C<sub>3</sub> alkyl or hydroxyalkyl group, for example methyl, ethyl, propyl, hydroxyethyl, and the like, poly(C<sub>2-3</sub> alkoxy), polyethoxy, benzyl, or mixtures thereof; each X is independently (CH<sub>2</sub>)<sub>n</sub>, CH<sub>2</sub>-CH(CH<sub>3</sub>)- or CH-(CH<sub>3</sub>)-CH<sub>2</sub>-; each Y may comprise —O—(O)C—, —C(O)O—, —NR—C(O)—, or —C(O)—NR—; each m is 2 or 3; each n is from 1 to about 4, in one aspect 2; the sum of carbons in each R<sup>1</sup>, plus one when Y is —O—(O)C— or —NR—C(O)—, may be C<sub>12</sub>-C<sub>22</sub>, or C<sub>14</sub>-C<sub>20</sub>, with each R<sup>1</sup> being a hydrocarbyl, or substituted hydrocarbyl group; and X<sup>-</sup> may comprise any softener-compatible anion. In one aspect, the softener-compatible anion may comprise chloride, bromide, methylsulfate, ethylsulfate, sulfate, and nitrate. In another aspect, the softener-compatible anion may comprise chloride or methyl sulfate.

In another aspect, the fabric softening active may comprise the general formula:



wherein each Y, R, R<sup>1</sup>, and X<sup>-</sup> have the same meanings as before. Such compounds include those having the formula:



wherein each R may comprise a methyl or ethyl group. In one aspect, each R<sup>1</sup> may comprise a C<sub>15</sub> to C<sub>19</sub> group. As used herein, when the diester is specified, it can include the monoester that is present.

These types of agents and general methods of making them are disclosed in U.S. Pat. No. 4,137,180. An example of a suitable DEQA (2) is the “propyl” ester quaternary ammonium fabric softener active comprising the formula 1,2-di(acyloxy)-3-trimethylammoniopropane chloride.

A third type of useful fabric softening active has the formula:



wherein each R, R<sup>1</sup>, m and X<sup>-</sup> have the same meanings as before.

In a further aspect, the fabric softening active may comprise the formula:



(4) 5

10

wherein each R, R<sup>1</sup>, and A<sup>-</sup> have the definitions given above; R<sup>2</sup> may comprise a C<sub>1-6</sub> alkylene group, in one aspect an ethylene group; and G may comprise an oxygen atom or an —NR— group;

In a yet further aspect, the fabric softening active may comprise the formula:



(5) 20

25

wherein R<sup>1</sup>, R<sup>2</sup> and G are defined as above.

In a further aspect, the fabric softening active may comprise condensation reaction products of fatty acids with dialkylenetriamines in, e.g., a molecular ratio of about 2:1, said reaction products containing compounds of the formula:



wherein R<sup>1</sup>, R<sup>2</sup> are defined as above, and R<sup>3</sup> may comprise a C<sub>1-6</sub> alkylene group, in one aspect, an ethylene group and wherein the reaction products may optionally be quaternized by the addition of an alkylating agent such as dimethyl sulfate. Such quaternized reaction products are described in additional detail in U.S. Pat. No. 5,296,622.

In a yet further aspect, the fabric softening active may comprise the formula:



wherein R, R<sup>1</sup>, R<sup>2</sup>, R<sup>3</sup> and A<sup>-</sup> are defined as above;

In a yet further aspect, the fabric softening active may comprise reaction products of fatty acid with hydroxyalkylalkylenediamines in a molecular ratio of about 2:1, said reaction products containing compounds of the formula:



wherein R<sup>1</sup>, R<sup>2</sup> and R<sup>3</sup> are defined as above;

In a yet further aspect, the fabric softening active may comprise the formula:



(9)

wherein R, R<sup>1</sup>, R<sup>2</sup>, and A<sup>-</sup> are defined as above.

In yet a further aspect, the fabric softening active may comprise the formula:

(10)



5

10

wherein:

X<sub>1</sub> is a C<sub>2-3</sub> alkyl group, in one aspect, an ethyl group; X<sub>2</sub> and X<sub>3</sub> are independently C<sub>1-6</sub> linear or branched alkyl or alkenyl groups, in one aspect, methyl, ethyl or isopropyl groups;

R<sub>1</sub> and R<sub>2</sub> are independently C<sub>8-22</sub> linear or branched alkyl or alkenyl groups; characterized in that;

A and B are independently selected from the group comprising —O—(C=O)—, —(C=O)—O—, or mixtures thereof, in one aspect, —O—(C=O)—

Non-limiting examples of fabric softening actives comprising formula (1) are N,N-bis(stearoyl-oxy-ethyl)-N,N-dimethyl ammonium chloride, N,N-bis(tallowoyl-oxy-ethyl)-N,N-dimethyl ammonium chloride, N,N-bis(stearoyl-oxy-ethyl)-N-(2-hydroxyethyl)-N-methyl ammonium methylsulfate.

Non-limiting examples of fabric softening actives comprising formula (2) is 1,2-di-(stearoyl-oxy)-3-trimethyl ammoniumpropane chloride.

Non-limiting examples of fabric softening actives comprising formula (3) include dialkylenedimethylammonium salts such as dicanoladimethylammonium chloride, di(hard) tallowdimethylammonium chloride, dicanoladimethylammonium methylsulfate, and mixtures thereof. An example of commercially available dialkylenedimethylammonium salts usable in the present invention is dioleyldimethylammonium chloride available from Witco Corporation under the trade name Adogen® 472 and dihardtallow dimethylammonium chloride available from Akzo Nobel Arquad 2HT75.

A non-limiting example of fabric softening actives comprising formula (4) is 1-methyl-1-stearoylamidoethyl-2-stearoylimidazolinium methylsulfate wherein R<sup>1</sup> is an acyclic aliphatic C<sub>15</sub>-C<sub>17</sub> hydrocarbon group, R<sup>2</sup> is an ethylene group, G is a NH group, R<sup>5</sup> is a methyl group and A<sup>-</sup> is a methyl sulfate anion, available commercially from the Witco Corporation under the trade name Varisoft®.

A non-limiting example of fabric softening actives comprising formula (5) is 1-tallowylamidoethyl-2-tallowylimidazoline wherein R<sup>1</sup> is an acyclic aliphatic C<sub>15</sub>-C<sub>17</sub> hydrocarbon group, R<sup>2</sup> is an ethylene group, and G is a NH group.

A non-limiting example of a fabric softening active comprising formula (6) is the reaction products of fatty acids with diethylenetriamine in a molecular ratio of about 2:1, said reaction product mixture containing N,N'-dialkyldiethylenetriamine with the formula:



wherein R<sup>1</sup> is an alkyl group of a commercially available fatty acid derived from a vegetable or animal source, such as Emersol® 223LL or Emersol® 7021, available from Henkel Corporation, and R<sup>2</sup> and R<sup>3</sup> are divalent ethylene groups.

In one aspect, said fatty acid may be obtained, in whole or in part, from a renewable source, via extraction from plant material, fermentation from plant material, and/or obtained via genetically modified organisms such as algae or yeast.

A non-limiting example of Compound (7) is a di-fatty amidoamine based softener having the formula:



wherein R<sup>1</sup> is an alkyl group. An example of such compound is that commercially available from the Witco Corporation e.g. under the trade name Varisoft® 222LT.

An example of a fabric softening active comprising formula (8) is the reaction products of fatty acids with N-2-hydroxyethylmethylenediamine in a molecular ratio of about 2:1, said reaction product mixture containing a compound of the formula:



wherein  $R^1-C(O)$  is an alkyl group of a commercially available fatty acid derived from a vegetable or animal source, such as Emersol® 223LL or Emersol® 7021, available from Henkel Corporation.

An example of a fabric softening active comprising formula (9) is the diquaternary compound having the formula:



wherein R<sup>1</sup> is derived from fatty acid. Such compound is available from Witco Company.

A non-limiting example of a fabric softening active comprising formula (10) is a dialkyl imidazoline diester compound, where the compound is the reaction product of N-(2-hydroxyethyl)-1,2-ethylenediamine or N-(2-hydroxyisopropyl)-1,2-ethylenediamine with glycolic acid, esterified with fatty acid, where the fatty acid is (hydrogenated) tallow fatty acid, palm fatty acid, hydrogenated palm fatty acid, oleic acid, rapeseed fatty acid, hydrogenated rapeseed fatty acid or a mixture of the above.

It will be understood that combinations of softener actives disclosed above are suitable for use in this invention.

### Anion A

In the cationic nitrogenous salts herein, the anion A<sup>-</sup>, which comprises any softener compatible anion, provides electrical neutrality. Most often, the anion used to provide electrical neutrality in these salts is from a strong acid, especially a halide, such as chloride, bromide, or iodide. However, other anions can be used, such as methylsulfate, ethylsulfate, acetate, formate, sulfate, carbonate, fatty acid anions and the like. In one aspect, the anion A may comprise chloride or methylsulfate. The anion, in some aspects, may carry a double charge. In this aspect, A<sup>-</sup> represents half a group.

In one embodiment, the fabric softening agent is chosen from at least one of the following: ditallowoyloxyethyl dimethyl ammonium chloride, dihydrogenated-tallowoyloxyethyl dimethyl ammonium chloride, ditallow dimethyl ammonium chloride, dihydrogenatedtallow dimethyl ammonium chloride, ditallowoyloxyethyl methylhydroxyethylammonium methyl sulfate, dihydrogenated-tallowoyloxyethyl methyl hydroxyethylammonium chloride, or combinations thereof.

## Sucrose Esters

Nonionic fabric care benefit agents can comprise sucrose esters, and are typically derived from sucrose and fatty acids. Sucrose ester is composed of a sucrose moiety having one or more of its hydroxyl groups esterified.

Sucrose is a disaccharide having the following formula:



Alternatively, the sucrose molecule can be represented by the formula:  $M(OH)_8$ , wherein M is the disaccharide backbone and there are total of 8 hydroxyl groups in the molecule.

Thus, sucrose esters can be represented by the following formula:



wherein x is the number of hydroxyl groups that are esterified, whereas (8-x) is the hydroxyl groups that remain unchanged; x is an integer selected from 1 to 8, alternatively from 2 to 8, alternatively from 3 to 8, or from 4 to 8; and R<sup>1</sup> moieties are independently selected from C<sub>1</sub>-C<sub>22</sub> alkyl or C<sub>1</sub>-C<sub>30</sub> alkoxy, linear or branched, cyclic or acyclic, saturated or unsaturated, substituted or unsubstituted.

In one embodiment, the R<sup>1</sup> moieties comprise linear alkyl or alkoxy moieties having independently selected and varying chain length. For example, R<sup>1</sup> may comprise a mixture of linear alkyl or alkoxy moieties wherein greater than about 35 20% of the linear chains are C<sub>18</sub>, alternatively greater than about 50% of the linear chains are C<sub>18</sub>, alternatively greater than about 80% of the linear chains are C<sub>18</sub>.

In another embodiment, the R<sup>1</sup> moieties comprise a mixture of saturate and unsaturated alkyl or alkoxy moieties; the degree of unsaturation can be measured by "Iodine Value" (hereinafter referred as "IV", as measured by the standard AOCS method). The IV of the sucrose esters suitable for use herein ranges from about 1 to about 150, or from about 2 to about 100, or from about 5 to about 85. The R<sup>1</sup> moieties may be hydrogenated to reduce the degree of unsaturation. In the case where a higher IV is preferred, such as from about 40 to about 95, then oleic acid and fatty acids derived from soybean oil and canola oil are the starting materials.

In a further embodiment, the unsaturated R<sup>1</sup> moieties may comprise a mixture of "cis" and "trans" forms about the unsaturated sites. The "cis"/"trans" ratios may range from about 1:1 to about 50:1, or from about 2:1 to about 40:1, or from about 3:1 to about 30:1, or from about 4:1 to about 20:1.

## 55 Dispersible Polyolefins

Generally, all dispersible polyolefins that provide fabric care benefits can be used as water insoluble fabric care benefit agents in the present invention. The polyolefins can be in the format of waxes, emulsions, dispersions or suspensions. Non-limiting examples are discussed below.

In one embodiment, the polyolefin is chosen from a polyethylene, polypropylene, or a combination thereof. The polyolefin may be at least partially modified to contain various functional groups, such as carboxyl, alkylamide, sulfonic acid or amide groups. In another embodiment, the polyolefin is at least partially carboxyl modified or, in other words, oxidized.

## 13

For ease of formulation, the dispersible polyolefin may be introduced as a suspension or an emulsion of polyolefin dispersed by use of an emulsifying agent. The polyolefin suspension or emulsion may comprise from about 1% to about 60%, alternatively from about 10% to about 55%, alternatively from 20% to about 50% by weight of polyolefin. The polyolefin may have a wax dropping point (see ASTM D3954-94, volume 15.04—"Standard Test Method for Dropping Point of Waxes") from about 20° to about 170° C., alternatively from about 50° to about 140° C. Suitable polyethylene waxes are available commercially from suppliers including but not limited to Honeywell (A-C polyethylene), Clariant (Velustrol® emulsion), and BASF (LUWAX®).

When an emulsion is employed with the dispersible polyolefin, the emulsifier may be any suitable emulsification agent. Non-limiting examples include an anionic, cationic, nonionic surfactant, or a combination thereof. However, almost any suitable surfactant or suspending agent may be employed as the emulsification agent. The dispersible polyolefin is dispersed by use of an emulsification agent in a ratio to polyolefin wax of about 1:100 to about 1:2, alternatively from about 1:50 to about 1:5, respectively.

## Polymer Latexes

Polymer latex is made by an emulsion polymerization which includes one or more monomers, one or more emulsifiers, an initiator, and other components familiar to those of ordinary skill in the art. Generally, all polymer latexes that provide fabric care benefits can be used as water insoluble fabric care benefit agents of the present invention. Additional non-limiting examples include the monomers used in producing polymer latexes such as: (1) 100% or pure butylacrylate; (2) butylacrylate and butadiene mixtures with at least 20% (weight monomer ratio) of butylacrylate; (3) butylacrylate and less than 20% (weight monomer ratio) of other monomers excluding butadiene; (4) alkylacrylate with an alkyl carbon chain at or greater than C<sub>6</sub>; (5) alkylacrylate with an alkyl carbon chain at or greater than C<sub>6</sub> and less than 50% (weight monomer ratio) of other monomers; (6) a third monomer (less than 20% weight monomer ratio) added into an aforementioned monomer systems; and (7) combinations thereof.

Polymer latexes that are suitable fabric care benefit agents in the present invention may include those having a glass transition temperature of from about -120° C. to about 120° C., alternatively from about -80° C. to about 60° C. Suitable emulsifiers include anionic, cationic, nonionic and amphoteric surfactants. Suitable initiators include initiators that are suitable for emulsion polymerization of polymer latexes. The particle size diameter ( $\chi_{50}$ ) of the polymer latexes can be from about 1 nm to about 10  $\mu$ m, alternatively from about 10 nm to about 1  $\mu$ m, or even from about 10 nm to about 20 nm.

## Fatty Acid

One aspect of the invention provides a fabric softening composition comprising a fatty acid, such as a free fatty acid. The term "fatty acid" is used herein in the broadest sense to include unprotonated or protonated forms of a fatty acid; and includes fatty acid that is bound or unbound to another chemical moiety as well as the various combinations of these species of fatty acid. One skilled in the art will readily appreciate that the pH of an aqueous composition will dictate, in part, whether a fatty acid is protonated or unprotonated. In another embodiment, the fatty acid is in its unprotonated, or salt form, together with a counter ion, such as, but not limited to, calcium, magnesium, sodium, potassium and the like. The term "free fatty acid" means a fatty

## 14

acid that is not bound to another chemical moiety (covalently or otherwise) to another chemical moiety.

In one embodiment, the fatty acid may include those containing from about 12 to about 25, from about 13 to about 22, or even from about 16 to about 20, total carbon atoms, with the fatty moiety containing from about 10 to about 22, from about 12 to about 18, or even from about 14 (mid-cut) to about 18 carbon atoms.

The fatty acids of the present invention may be derived from (1) an animal fat, and/or a partially hydrogenated animal fat, such as beef tallow, lard, etc.; (2) a vegetable oil, and/or a partially hydrogenated vegetable oil such as canola oil, safflower oil, peanut oil, sunflower oil, sesame seed oil, rapeseed oil, cottonseed oil, corn oil, soybean oil, tall oil, rice bran oil, palm oil, palm kernel oil, coconut oil, other tropical palm oils, linseed oil, tung oil, etc.; (3) processed and/or bodied oils, such as linseed oil or tung oil via thermal, pressure, alkali-isomerization and catalytic treatments; (4) a mixture thereof, to yield saturated (e.g. stearic acid), unsaturated (e.g. oleic acid), polyunsaturated (linoleic acid), branched (e.g. isostearic acid) or cyclic (e.g. saturated or unsaturated  $\alpha$ -disubstituted cyclopentyl or cyclohexyl derivatives of polyunsaturated acids) fatty acids.

Mixtures of fatty acids from different fat sources can be used.

In one aspect, at least a majority of the fatty acid that is present in the fabric softening composition of the present invention is unsaturated, e.g., from about 40% to 100%, from about 55% to about 99%, or even from about 60% to about 98%, by weight of the total weight of the fatty acid present in the composition, although fully saturated and partially saturated fatty acids can be used. As such, the total level of polyunsaturated fatty acids (TPU) of the total fatty acid of the inventive composition may be from about 0% to about 75% by weight of the total weight of the fatty acid present in the composition.

The cis/trans ratio for the unsaturated fatty acids may be important, with the cis/trans ratio (of the C18:1 material) being from at least about 1:1, at least about 3:1, from about 4:1 or even from about 9:1 or higher.

Branched fatty acids such as isostearic acid are also suitable since they may be more stable with respect to oxidation and the resulting degradation of color and odor quality.

The Iodine Value or "IV" measures the degree of unsaturation in the fatty acid. In one embodiment of the invention, the fatty acid has an IV from about 10 to about 140, from about 15 to about 100 or even from about 15 to about 60.

Another class of fatty ester fabric care actives is softening oils, which include but are not limited to, vegetable oils (such as soybean, sunflower, and canola), hydrocarbon based oils (natural and synthetic petroleum lubricants, in one aspect polyolefins, isoparaffins, and cyclic paraffins), triolein, fatty esters, fatty alcohols, fatty amines, fatty amides, and fatty ester amines. Oils can be combined with fatty acid softening agents, clays, and silicones.

## Clays

In one embodiment of the invention, the fabric care composition may comprise a clay as a fabric care active. In one embodiment clay can be a softener or co-softeners with another softening active, for example, silicone. Suitable clays include those materials classified geologically smectites.

## Silicone

In one embodiment, the fabric softening composition comprises a silicone. Suitable levels of silicone may comprise from about 0.1% to about 70%, alternatively from

## 15

about 0.3% to about 40%, alternatively from about 0.5% to about 30%, alternatively from about 1% to about 20% by weight of the composition. Useful silicones can be any silicone comprising compound. In one embodiment, the silicone polymer is selected from the group consisting of cyclic silicones, polydimethylsiloxanes, aminosilicones, cationic silicones, silicone polyethers, silicone resins, silicone urethanes, and mixtures thereof. In one embodiment, the silicone is a polydialkylsilicone, alternatively a polydimethyl silicone (polydimethyl siloxane or "PDMS"), or a derivative thereof. In another embodiment, the silicone is chosen from an aminofunctional silicone, amino-polyether silicone, alkyloxyated silicone, cationic silicone, ethoxyated silicone, propoxylated silicone, ethoxyated/propoxylated silicone, quaternary silicone, or combinations thereof.

In another embodiment, the silicone may be chosen from a random or blocky organosilicone polymer having the following formula:



wherein:

j is an integer from 0 to about 98; in one aspect j is an integer from 0 to about 48; in one aspect, j is 0;

k is an integer from 0 to about 200, in one aspect k is an integer from 0 to about 50; when k=0, at least one of  $R_1, R_2$  or  $R_3$  is  $-X-Z$ ;

m is an integer from 4 to about 5,000; in one aspect m is an integer from about 10 to about 4,000; in another aspect m is an integer from about 50 to about 2,000;

$R_1, R_2$  and  $R_3$  are each independently selected from the group consisting of H, OH,  $C_1-C_{32}$  alkyl,  $C_1-C_{32}$  substituted alkyl,  $C_5-C_{32}$  or  $C_6-C_{32}$  aryl,  $C_1-C_{32}$  or  $C_6-C_{32}$  substituted aryl,  $C_6-C_{32}$  alkylaryl,  $C_6-C_{32}$  substituted alkylaryl,  $C_1-C_{32}$  alkoxy,  $C_1-C_{32}$  substituted alkoxy and  $X-Z$ ;

each  $R_4$  is independently selected from the group consisting of H, OH,  $C_1-C_{32}$  alkyl,  $C_1-C_{32}$  substituted alkyl,  $C_5-C_{32}$  or  $C_6-C_{32}$  aryl,  $C_5-C_{32}$  or  $C_6-C_{32}$  substituted aryl,  $C_6-C_{32}$  alkylaryl,  $C_6-C_{32}$  substituted alkylaryl,  $C_1-C_{32}$  alkoxy and  $C_1-C_{32}$  substituted alkoxy;

each X in said alkyl siloxane polymer comprises a substituted or unsubstituted divalent alkylene radical comprising 2-12 carbon atoms, in one aspect each divalent alkylene radical is independently selected from the group consisting of  $-(CH_2)_s-$  wherein s is an integer from about 2 to about 8, from about 2 to about 4; in one aspect, each X in said alkyl siloxane polymer comprises a substituted divalent alkylene radical selected from the group consisting of:  $-CH_2-CH(OH)-CH_2-$ ;  $-CH_2-CH_2-CH(OH)-$ ; and



each Z is selected independently from the group consisting of



## 16

-continued



with the proviso that when Z is a quat, Q cannot be an amide, imine, or urea moiety and if Q is an amide, imine, or urea moiety, then any additional Q bonded to the same nitrogen as said amide, imine, or urea moiety must be H or a  $C_1-C_6$  alkyl, in one aspect, said additional Q is H; for Z  $A''-$  is a suitable charge balancing anion. In one aspect  $A''-$  is selected from the group consisting of  $\text{Cl}^-$ ,  $\text{Br}^-$ ,  $\text{I}^-$ , methylsulfate, toluene sulfonate, carboxylate and phosphate; and at least one Q in said organosilicone is independently selected from  $-\text{CH}_2-\text{CH}(\text{OH})-\text{CH}_2-\text{R}_5$ ;





wherein each  $R_5$  is independently selected from the group consisting of H,  $C_1$ - $C_{32}$  alkyl,  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl,  $C_6$ - $C_{32}$  substituted alkylaryl,  $-(CHR_6-CHR_6-O)_w-L$  and a siloxyl residue;

each  $R_6$  is independently selected from H,  $C_1$ - $C_{18}$  alkyl each L is independently selected from  $-C(O)-R_7$  or  $R_7$ ;

w is an integer from 0 to about 500, in one aspect w is an integer from about 1 to about 200; in one aspect w is an integer from about 1 to about 50;

each  $R_7$  is selected independently from the group consisting of H;  $C_1$ - $C_{32}$  alkyl;  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl;  $C_6$ - $C_{32}$  substituted alkylaryl and a siloxyl residue;

each T is independently selected from H, and



and

wherein each v in said organosilicone is an integer from 1 to about 10, in one aspect, v is an integer from 1 to about 5 and the sum of all v indices in each Q in the said organosilicone is an integer from 1 to about 30 or from 1 to about 20 or even from 1 to about 10.

In another embodiment, the silicone may be chosen from a random or blocky organosilicone polymer having the following formula:



wherein

j is an integer from 0 to about 98; in one aspect j is an integer from 0 to about 48; in one aspect, j is 0; k is an integer from 0 to about 200; when k=0, at least one of  $R_1$ ,  $R_2$  or  $R_3$ —X—Z, in one aspect, k is an integer from 0 to about 50

m is an integer from 4 to about 5,000; in one aspect m is an integer from about 10 to about 4,000; in another aspect m is an integer from about 50 to about 2,000;  $R_1$ ,  $R_2$  and  $R_3$  are each independently selected from

the group consisting of H, OH,  $C_1$ - $C_{32}$  alkyl,  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl,  $C_6$ - $C_{32}$  substituted alkylaryl,  $C_1$ - $C_{32}$  alkoxy,  $C_1$ - $C_{32}$  substituted alkoxy and X—Z;

each  $R_4$  is independently selected from the group consisting of H, OH,  $C_1$ - $C_{32}$  alkyl,  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl,  $C_6$ - $C_{32}$  substituted alkylaryl,  $C_1$ - $C_{32}$  alkoxy and  $C_1$ - $C_{32}$  substituted alkoxy;

each X comprises of a substituted or unsubstituted divalent alkylene radical comprising 2-12 carbon atoms; in one aspect each X is independently selected from the group consisting of  $-(CH_2)_s-O-$ ;  $-(CH_2-CH(OH)-CH_2-O-$ ;



wherein each s independently is an integer from about 2 to about 8, in one aspect s is an integer from about 2 to about 4;

At least one Z in the said organosiloxane is selected from the group consisting of  $R_5$ ;



19



provided that when  $X$  is



then  $Z = -OR_s$  or



wherein  $A^-$  is a suitable charge balancing anion. In one aspect  $A^-$  is selected from the group consisting of  $Cl^-$ ,  $Br^-$ .

$\text{I}^-$ , methylsulfate, toluene sulfonate, carboxylate and phosphate and

each additional Z in said organosilicone is independently selected from the group comprising of H, C<sub>1</sub>-C<sub>32</sub> alkyl, C<sub>1</sub>-C<sub>32</sub> substituted alkyl, C<sub>5</sub>-C<sub>32</sub> or C<sub>6</sub>-C<sub>32</sub> aryl, C<sub>5</sub>-C<sub>32</sub> or C<sub>6</sub>-C<sub>32</sub> substituted aryl, C<sub>6</sub>-C<sub>32</sub> alkylaryl, C<sub>6</sub>-C<sub>32</sub> substituted alkylaryl, R<sub>5</sub>,



20

-continued



provided that when  $X$  is



then  $Z = -OR_s$  or



each  $R_5$  is independently selected from the group consisting of H;  $C_1$ - $C_{32}$  alkyl;  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl or  $C_6$ - $C_{32}$  alkylaryl, or  $C_6$ - $C_{32}$

substituted alkylaryl,  
 $-(\text{CHR}_6-\text{CHR}_6-\text{O})_w-\text{CHR}_6-\text{CHR}_6-\text{L}$  and  
 siloxyl residue wherein each L is independently  
 selected from  $\text{O}$ ,  $\text{C}(\text{O})$ ,  $\text{R}$  or  $\text{O}-\text{R}$ .



w is an integer from 0 to about 500, in one aspect w is an integer from 0 to about 200, one aspect w is an integer from 0 to about 50;

each  $R_6$  is independently selected from H or  $C_1-C_{18}$  alkyl;

each  $R_7$  is independently selected from the group consisting of H;  $C_1$ - $C_{32}$  alkyl;  $C_1$ - $C_{32}$  substituted alkyl,  $C_5$ - $C_{32}$  or  $C_6$ - $C_{32}$  aryl,  $C_5$ - $C_{32}$  or  $C_6$ - $C_{32}$  substituted aryl,  $C_6$ - $C_{32}$  alkylaryl, and  $C_6$ - $C_{32}$  substituted aryl, and a siloxyl residue;

each  $T$  is independently selected from  $H$ ;



wherein each v in said organosilicone is an integer from 1 to about 10, in one aspect, v is an integer from 1 to about 5 and the sum of all v indices in each Z in the said organosilicone is an integer from 1 to about 30 or from 1 to about 20 or even from 1 to about 10.

In one embodiment, the silicone is one comprising a relatively high molecular weight. A suitable way to describe the molecular weight of a silicone includes describing its viscosity. A high molecular weight silicone is one having a viscosity of from about 10 cSt to about 3,000,000 cSt, or from about 100 cSt to about 1,000,000 cSt, or from about 1,000 cSt to about 600,000 cSt, or even from about 6,000 cSt to about 300,000 cSt.

In one embodiment, the silicone comprises a blocky 15 cationic organopolysiloxane having the formula:



wherein:

$M=[SiR_1R_2R_3O_{1/2}]$ ,  $[SiR_1R_2G_1O_{1/2}]$ ,  $[SiR_1G_1G_2O_{1/2}]$ ,  $[SiG_1G_2G_3O_{1/2}]$ , or combinations thereof;

$D=[SiR_1R_2O_{2/2}]$ ,  $[SiR_1G_1O_{2/2}]$ ,  $[SiG_1G_2O_{2/2}]$  or combinations thereof;

$T=[SiR_1O_{3/2}]$ ,  $[SiG_1O_{3/2}]$  or combinations thereof;

$Q=[SiO_{4/2}]$ ;

w is an integer from 1 to  $(2+y+2z)$ ;

x is an integer from 5 to 15,000;

y is an integer from 0 to 98;

z is an integer from 0 to 98;

$R_1$ ,  $R_2$  and  $R_3$  are each independently selected from the group consisting of H, OH,  $C_1-C_{32}$  alkyl,  $C_1-C_{32}$  substituted alkyl,  $C_5-C_{32}$  or  $C_6-C_{32}$  aryl,  $C_5-C_{32}$  or  $C_6-C_{32}$  substituted aryl,  $C_6-C_{32}$  alkylaryl,  $C_6-C_{32}$  substituted alkylaryl,  $C_1-C_{32}$  alkoxy,  $C_1-C_{32}$  substituted alkoxy,  $C_1-C_{32}$  alkylamino, and  $C_1-C_{32}$  substituted alkylamino;

at least one of M, D, or T incorporates at least one moiety  $G_1$ ,  $G_2$  or  $G_3$ ; and  $G_1$ ,  $G_2$ , and  $G_3$  are each independently selected from the formula:



wherein:

X comprises a divalent radical selected from the group consisting of  $C_1-C_{32}$  alkylene,  $C_1-C_{32}$  substituted alkylene,  $C_5-C_{32}$  or  $C_6-C_{32}$  arylene,  $C_5-C_{32}$  or  $C_6-C_{32}$  substituted arylene,  $C_6-C_{32}$  arylalkylene,  $C_6-C_{32}$  substituted arylalkylene,  $C_1-C_{32}$  alkoxy,  $C_1-C_{32}$  substituted alkoxy,  $C_1-C_{32}$  alkyleneamino,  $C_1-C_{32}$  substituted alkyleneamino, ring-opened epoxide, and ring-opened glycidyl, with the proviso that if X does not comprise a repeating alkylene oxide moiety then X can further comprise a heteroatom selected from the group consisting of P, N and O;

each  $R_4$  comprises identical or different monovalent radicals selected from the group consisting of H,  $C_1-C_{32}$  alkyl,  $C_1-C_{32}$  substituted alkyl,  $C_5-C_{32}$  or  $C_6-C_{32}$  aryl,  $C_5-C_{32}$  or  $C_6-C_{32}$  substituted aryl,  $C_6-C_{32}$  alkylaryl, and  $C_6-C_{32}$  substituted alkylaryl;

E comprises a divalent radical selected from the group consisting of  $C_1-C_{32}$  alkylene,  $C_1-C_{32}$  substituted alkylene,  $C_5-C_{32}$  or  $C_6-C_{32}$  arylene,  $C_5-C_{32}$  or  $C_6-C_{32}$  substituted arylene,  $C_6-C_{32}$  arylalkylene,  $C_6-C_{32}$  substituted arylalkylene,  $C_1-C_{32}$  alkoxy,  $C_1-C_{32}$  substituted alkoxy,  $C_1-C_{32}$  alkyleneamino,  $C_1-C_{32}$  substituted alkyleneamino, ring-opened epoxide and ring-opened glycidyl, with the proviso that if E

does not comprise a repeating alkylene oxide moiety then E can further comprise a heteroatom selected from the group consisting of P, N, and O;

5 E' comprises a divalent radical selected from the group consisting of  $C_1-C_{32}$  alkylene,  $C_1-C_{32}$  substituted alkylene,  $C_5-C_{32}$  or  $C_6-C_{32}$  arylene,  $C_5-C_{32}$  or  $C_6-C_{32}$  substituted arylene,  $C_6-C_{32}$  arylalkylene,  $C_6-C_{32}$  substituted arylalkylene,  $C_1-C_{32}$  alkoxy,  $C_1-C_{32}$  substituted alkoxy,  $C_1-C_{32}$  alkyleneamino,  $C_1-C_{32}$  substituted alkyleneamino, ring-opened epoxide and ring-opened glycidyl, with the proviso that if E' does not comprise a repeating alkylene oxide moiety then E' can further comprise a heteroatom selected from the group consisting of P, N, and O;

10 p is an integer independently selected from 1 to 50; n is an integer independently selected from 1 or 2; when at least one of  $G_1$ ,  $G_2$ , or  $G_3$  is positively charged,  $A^{-t}$  is a suitable charge balancing anion or anions such that the total charge, k, of the charge-balancing anion or anions is equal to and opposite from the net charge on the moiety  $G_1$ ,  $G_2$  or  $G_3$ ; wherein t is an integer independently selected from 1, 2, or 3; and  $k \leq (p^*2/t)+1$ ; such that the total number of cationic charges balances the total number of anionic charges in the organopolysiloxane molecule; and wherein at 15 least one E does not comprise an ethylene moiety.

#### Process of Making Synthetic Polymers

The polymer, in one aspect, comprises from 0.001% to 10% by weight of the fabric care composition. In alternative aspects, the polymer comprises from 0.01% to 0.5%, alternatively from 0.05% to 0.25%, alternatively from 0.1% to 0.20%, alternatively combinations thereof, of the polymer by weight of the fabric care composition.

30 Polymers useful in the present invention can be made by one skilled in the art. Examples of processes for making polymers include, but are not limited, solution polymerization, emulsion polymerization, inverse emulsion polymerization, inverse dispersion polymerization, and liquid dispersion polymer technology. In one aspect, a method of 35 making a polymer having a chain transfer agent (CTA) value in a range of less than 10,000 ppm by weight of the polymer, preferably 5 ppm to 5,000 ppm, more preferably 50 to 1,000 ppm is disclosed. Another aspect of the invention is directed to providing a polymer having a cross linker greater than 5 40 ppm, alternatively greater than 45 ppm, by weight of the polymer.

45 In one aspect of making a polymer, the CTA is present in a range greater than about 100 ppm based on the weight of the polymer. In one aspect, the CTA is from about 100 ppm to about 10,000 ppm, alternatively from about 500 ppm to about 4,000 ppm, alternatively from about 1,000 ppm to about 3,500 ppm, alternatively from about 1,500 ppm to about 3,000 ppm, alternatively from about 1,500 ppm to about 2,500 ppm, alternatively combinations thereof based 50 on the weight of the polymer. In yet another aspect, the CTA is greater than about 1,000 based on the weight of the polymer. It is also suitable to use mixtures of chain transfer agents.

55 In one aspect of the invention, the polymer comprises 5-100% by weight (wt-%) of at least one cationic monomer and 5-95 wt-% of at least one non-ionic monomer. The weight percentages relate to the total weight of the copolymer. In another aspect of the invention, the polymer comprises 0-50% by weight (wt-%) of an anionic monomer.

#### Cationic Monomers for Synthetic Polymers

Suitable cationic monomers include dialkyl ammonium halides or compounds according to formula (I):



wherein:

$\text{R}_1$  is chosen from hydrogen, or  $\text{C}_1\text{-C}_4$  alkyl, in one aspect,  $\text{R}_1$  is hydrogen or methyl;

$\text{R}_2$  is chosen from hydrogen or methyl, in one aspect,  $\text{R}_1$  is hydrogen

$\text{R}_3$  is chosen from  $\text{C}_1\text{-C}_4$  alkylene, in one aspect,  $\text{R}_3$  is ethylene;

$\text{R}_4$ ,  $\text{R}_5$ , and  $\text{R}_6$  are each independently chosen from hydrogen,  $\text{C}_1\text{-C}_4$  alkyl,  $\text{C}_1\text{-C}_4$  alkyl alcohol, or  $\text{C}_1\text{-C}_4$  alkoxy, in one aspect,  $\text{R}_4$ ,  $\text{R}_5$ , and  $\text{R}_6$  are methyl;

$\text{X}$  is chosen from  $-\text{O}-$ , or  $-\text{NH}-$ , in one aspect,  $\text{X}$  is  $-\text{O}-$ ; and

$\text{Y}$  is chosen from Cl, Br, I, hydrogensulfate or methysulfate, in one aspect,  $\text{Y}$  is Cl.

The alkyl and alkoxy groups may be linear or branched. The alkyl groups are methyl, ethyl, propyl, butyl, and isopropyl.

In one aspect, the cationic monomer of formula (I) is dimethyl aminoethyl acrylate methyl chloride. In another aspect, the cationic monomer of formula (I) is dimethyl aminoethyl methacrylate methyl chloride.

In another aspect, the cationic monomer is dialkyldimethyl ammonium chloride.

#### Non-Ionic Monomers for Synthetic Polymers

Suitable non-ionic monomers include compounds of formula (II) wherein



wherein:

$\text{R}_7$  is chosen from hydrogen or  $\text{C}_1\text{-C}_4$  alkyl; in one aspect  $\text{R}_7$  is hydrogen;

$\text{R}_8$  is chosen from hydrogen or methyl; in one aspect,  $\text{R}_8$  is hydrogen; and

$\text{R}_9$  and  $\text{R}_{10}$  are each independently chosen from hydrogen or  $\text{C}_1\text{-C}_4$  alkyl,  $\text{C}_1\text{-C}_4$  alkyl alcohol or  $\text{C}_1\text{-C}_4$  alkoxy; in one aspect,  $\text{R}_9$  and  $\text{R}_{10}$  are each independently chosen from hydrogen or methyl.

In one aspect, the non-ionic monomer is acrylamide.

In another aspect, the non-ionic monomer is hydroxyethyl acrylate.

#### Anionic Monomers for Synthetic Polymers

Suitable anionic monomer may include the group consisting of acrylic acid, methacrylic acid, itaconic acid, crotonic acid, maleic acid, fumaric acid, as well as monomers performing a sulfonic acid or phosphonic acid functions, such as 2-acrylamido-2-methyl propane sulfonic acid (ATBS), and their salts.

#### Cross-Linking Agent for Synthetic Polymers

The cross-linking agent contains at least two ethylenically unsaturated moieties. In one aspect, the cross-linking agent contains at least two or more ethylenically unsaturated moieties; in one aspect, the cross-linking agent contains at

least three or more ethylenically unsaturated moieties. Suitable cross-linking agents include 1,2,4-trivinylcyclohexane 1,7-octadiene, allyl acrylates and methacrylates, allyl-acrylamides and allyl-methacrylamides, allyl-acrylamides and allyl-methacrylamides, bisacrylamidoacetic acid, bisacrylamidoacetic acid, butadiene diacrylates and dimethacrylates of glycols and polyglycols,  $\text{N},\text{N}'\text{-methylene-bisacrylamide}$  and polyol polyallyl ethers, such as polyallylsaccharose and pentaerythrol triallyl ether, tetraallyl ammonium chloride, di(ethylene glycol) diacrylate, di(ethylene glycol) dimethacrylate, divinyl benzene, ethylene glycol diacrylate, ethylene glycol dimethacrylate,  $\text{N},\text{N}'\text{-}(1,2\text{-dihydroxyethylene})$  bisacrylamide, tetra(ethylene glycol) diacrylate, tri(ethylene glycol) dimethacrylate and mixtures thereof. A preferred cross-linking agent is tetraallyl ammonium chloride.

When Polymer 1 comprises a cationic vinyl addition monomer, the crosslinker(s) is (are) included in the range of from about 45 ppm to about 5,000 ppm, alternatively from about 50 ppm to about 500 ppm; alternatively from about 100 ppm to about 400 ppm, alternatively from about 500 ppm to about 4,500 ppm, alternatively from about 550 ppm to about 4,000 ppm based on the weight of the polymer.

When Polymer 2, comprises a cationic vinyl addition monomer the crosslinker(s) is (are) included in the range from 0 ppm to about 40 ppm, alternatively from about 0 ppm to about 20 ppm; alternatively from about 0 ppm to about 10 ppm based on the weight of the polymer.

#### Chain Transfer Agent (CTA) for Synthetic Polymers

The chain transfer agent includes mercaptans, malic acid, lactic acid, formic acid, isopropanol and hypophosphites, and mixtures thereof. In one aspect, the CTA is formic acid.

The CTA is present in a range greater than about 100 ppm based on the weight of the polymer. In one aspect, the CTA is present from about 100 ppm to about 10,000 ppm, alternatively from about 500 ppm to about 4,000 ppm, alternatively from about 1,000 ppm to about 3,500 ppm, alternatively from about 1,500 ppm to about 3,000 ppm, alternatively from about 1,500 ppm to about 2,500 ppm, alternatively combinations thereof based on the weight of the polymer. In yet another aspect, the CTA level is greater than about 1,000 based on the weight of the polymer. It is also suitable to use mixtures of chain transfer agents.

#### Polysaccharides for Polymer One

One aspect of the invention provides a fabric softener composition that comprises a polymer based on one or more sugar monomers, commonly called polysaccharides. Polysaccharides can be isolates from terrestrial and marine plants or are the exogenous metabolites of some bacteria; modified by partial organic synthesis, or the product of biochemical synthesis. One aspect of the invention provides a fabric softener composition that comprises a cationic modified polysaccharides.

In one embodiment the cationic polymer contains cationic nitrogen-containing moieties such as quaternary ammonium or cationic protonated amino moieties. The cationic protonated amines can be primary, secondary, or tertiary amines (preferably secondary or tertiary), depending upon the particular species. The average molecular weight of the cationic polymer is between about 10 million and about 5,000, preferably at least about 100,000, more preferably at least about 200,000, but preferably not more than about 2 million, more preferably not more than about 1.5 million.

The polymers also have a cationic charge density ranging from about 0.2 meq/gm to about 5 meq/gm, preferably at least about 0.4 meq/gm, more preferably at least about 0.6 meq/gm, but also preferably less than about 3 meq/gm, more

preferably less than about 2 meq/gm, at the pH of intended use of the fabric softening composition. The charge density can be controlled and adjusted in accordance with techniques well known in the art. As used herein the "charge density" of the cationic polymers is defined as the number of cationic sites per polymer gram atomic weight (molecular weight), and can be expressed in terms of meq/gm of cationic charge.

Any anionic counterions can be used in association with the cationic polymers so long as the polymers remain soluble in water, or in the fabric softening composition, and so long as the counterions are physically and chemically compatible with the essential components of the fabric softening composition or do not otherwise unduly impair product performance, stability or aesthetics. Nonlimiting examples of such counterions include halides (e.g., chlorine, fluorine, bromine, iodine), sulfate and methylsulfate.

The cationic nitrogen-containing moiety of the cationic deposition polymer is generally present as a substituent on all, or more typically on some, of the monomer units thereof. Thus, the cationic deposition polymer for use in the fabric softening composition includes homopolymers, copolymers, terpolymers, and so forth, of quaternary ammonium or cationic amine-substituted monomer units, optionally in combination with non-cationic monomers referred to herein as spacer monomers.

Any anionic counterions can be used in association with the cationic polymers so long as the polymers remain soluble in water, or in the fabric softening composition, and so long as the counterions are physically and chemically compatible with the essential components of the fabric softening composition or do not otherwise unduly impair product performance, stability or aesthetics. Nonlimiting examples of such counterions include halides (e.g., chlorine, fluorine, bromine, iodine), sulfate and methylsulfate.

The cationic nitrogen-containing moiety of the cationic deposition polymer is generally present as a substituent on all, or more typically on some, of the monomer units thereof. Thus, the cationic deposition polymer for use in the fabric softening composition includes homopolymers, copolymers, terpolymers, and so forth, of quaternary ammonium or cationic amine-substituted monomer units, optionally in combination with non-cationic monomers referred to herein as spacer monomers.

Suitable cationic polymers include cationic guar polymers such as; the JAGUAR® series of polymers from Rhodia, cationic cellulose derivatives such as CELQUATS® from Akzo Nobel, UCARE® polymers from the Dow Chemical Company, cationic starches, for example cationic potato starch TOPFAX from Avebe, C\* bond polymers series from Cargill, POLYGEL polymers K 100 and FLOCAID® series of polymers from Ingredion and cationic chitosan derivatives. It is preferred that the cationic polymer is selected from cationic starch, cationic cellulose, cationic guar, cationic chitosan derivatives polymers. Polysaccharides described can be selected from cassia, hyaluronan, konjac glucomannan, xyloglucan, kappa-carrageenan, gellan gum, succinoglycan, xanthan, curdlan and schizophylan.

#### Polysaccharides for Polymer Two

One aspect of the invention provides a fabric softener composition that comprises a polymer based on one or more sugar monomers, commonly called polysaccharides. Polysaccharides can be isolates from terrestrial and marine plants or are the exogenous metabolites of some bacteria; modified by partial organic synthesis, or the product of biochemical

synthesis. One aspect of the invention provides a fabric softener composition that comprises a cationic modified polysaccharides.

The cationic polymers may be present in the compositions in an amount of 0.01 to 5% by weight based upon the total weight of the composition, more preferably 0.02-3.5%, such as 0.5-2.5%.

In one embodiment the cationic polymer contains cationic nitrogen-containing moieties such as quaternary ammonium or cationic protonated amino moieties. The cationic protonated amines can be primary, secondary, or tertiary amines (preferably secondary or tertiary), depending upon the particular species. The average molecular weight of the cationic polymer is between about 10 million and about 5,000, preferably at least about 100,000, more preferably at least about 200,000, but preferably not more than about 2 million, more preferably not more than about 1.5 million.

The polymers also have a cationic charge density ranging from about 0.2 meq/gm to about 5 meq/gm, preferably at least about 0.4 meq/gm, more preferably at least about 0.6 meq/gm, but also preferably less than about 3 meq/gm, more preferably less than about 2 meq/gm, at the pH of intended use of the fabric softening composition. The charge density can be controlled and adjusted in accordance with techniques well known in the art. As used herein the "charge density" of the cationic polymers is defined as the number of cationic sites per polymer gram atomic weight (molecular weight), and can be expressed in terms of meq/gm of cationic charge.

Any anionic counterions can be used in association with the cationic polymers so long as the polymers remain soluble in water, or in the fabric softening composition, and so long as the counterions are physically and chemically compatible with the essential components of the fabric softening composition or do not otherwise unduly impair product performance, stability or aesthetics. Nonlimiting examples of such counterions include halides (e.g., chlorine, fluorine, bromine, iodine), sulfate and methylsulfate.

The cationic nitrogen-containing moiety of the cationic deposition polymer is generally present as a substituent on all, or more typically on some, of the monomer units thereof. Thus, the cationic deposition polymer for use in the fabric softening composition includes homopolymers, copolymers, terpolymers, and so forth, of quaternary ammonium or cationic amine-substituted monomer units, optionally in combination with non-cationic monomers referred to herein as spacer monomers.

Any anionic counterions can be used in association with the cationic polymers so long as the polymers remain soluble in water, or in the fabric softening composition, and so long as the counterions are physically and chemically compatible with the essential components of the fabric softening composition or do not otherwise unduly impair product performance, stability or aesthetics. Nonlimiting examples of such counterions include halides (e.g., chlorine, fluorine, bromine, iodine), sulfate and methylsulfate.

The cationic nitrogen-containing moiety of the cationic deposition polymer is generally present as a substituent on all, or more typically on some, of the monomer units thereof. Thus, the cationic deposition polymer for use in the fabric softening composition includes homopolymers, copolymers, terpolymers, and so forth, of quaternary ammonium or cationic amine-substituted monomer units, optionally in combination with non-cationic monomers referred to herein as spacer monomers.

In one embodiment, such fabric softening compositions comprise cationic starch at a level of from about 0.1% to

about 7%, alternatively from about 0.1% to about 5%, alternatively from about 0.3% to about 3%, and alternatively from about 0.5% to about 2.0%, by weight of the composition. Cationic starch is described in U.S. Pat. Pub. 2004/0204337 A1, published Oct. 14, 2004, to Corona et al., at paragraphs 16-32. Suitable cationic starches for use in the present compositions are commercially-available from Cargill under the trade name C\*BOND® and from Ingredion under the trade name CATO®, EchoPro® and Optipro.® In one embodiment, such fabric softening compositions comprise cellulose derivatives, for example, hydroxypropylmethyl celluloses, hydroxyethyl celluloses, methyl celluloses, carboxymethyl celluloses. In one embodiment, such fabric softening compositions comprise cellulose derivatives that are cationically modified. In one embodiment, such fabric softening compositions comprise cationic guar gum derivatives.

Preferred cationic cellulose polymers are the salts of hydroxyethyl cellulose reacted with trimethyl ammonium substituted epoxide, referred to in the industry (CTFA) as Polyquaternium 10 which are available from Amerchol Corp. (Edison, N.J., USA) in their Polymer JR and LR series of polymers with the most preferred being JR30M. Other suitable cationic polymers include cationic guar gum derivatives, such as guar hydroxypropyltrimonium chloride, specific examples of which include the Jaguar series (preferably Jaguar C-17) commercially available from Rhone-Poulenc Incorporated.

#### Molecular Weight Range for Polymers

In one aspect, the polymer comprises a Number Average Molecular Weight ( $M_n$ ) from about 10,000 Daltons to about 15,000,000 Daltons, alternatively from about 1,500,000 Daltons to about 2,500,000 Daltons.

In another aspect, the polymer comprises a Weight Average Molecular Weight ( $M_w$ ) from about 4,000,000 Daltons to about 11,000,000 Daltons, alternatively from about 4,000,000 Daltons to about 6,000,000 Daltons.

#### Adjunct Materials

While not essential for the purposes of the present invention, the non-limiting list of adjuncts illustrated hereinafter are suitable for use in the instant compositions and may be desirably incorporated in certain aspects of the invention, for example to assist or enhance cleaning performance, for treatment of the substrate to be cleaned, or to modify the aesthetics of the composition as is the case with perfumes, colorants, dyes or the like. The precise nature of these additional components, and levels of incorporation thereof, will depend on the physical form of the composition and the nature of the fabric treatment operation for which it is to be used. Suitable adjunct materials include, but are not limited to, surfactants, builders, chelating agents, dye transfer inhibiting agents, dispersants, enzymes, and enzyme stabilizers, catalytic materials, bleach activators, hydrogen peroxide, sources of hydrogen peroxide, preformed peracids, polymeric dispersing agents, clay soil removal/anti-redeposition agents, brighteners, suds suppressors, dyes, hueing dyes, perfumes, perfume delivery systems, structure elasticizing agents, carriers, structurants, hydrotropes, processing aids, solvents and/or pigments.

As stated, the adjunct ingredients are not essential to Applicants' compositions. Thus, certain aspects of Applicants' compositions do not contain one or more of the following adjuncts materials: surfactants, builders, chelating agents, dye transfer inhibiting agents, dispersants, enzymes, and enzyme stabilizers, catalytic materials, bleach activators, hydrogen peroxide, sources of hydrogen peroxide, preformed peracids, polymeric dispersing agents, clay soil

removal/anti-redeposition agents, brighteners, suds suppressors, dyes, hueing dyes, perfumes, perfume delivery systems structure elasticizing agents, carriers, hydrotropes, processing aids, solvents and/or pigments. However, when one or more adjuncts are present, such one or more adjuncts may be present as detailed below.

#### Hueing Dye—

The liquid laundry detergent composition may comprise a hueing dye. The hueing dyes employed in the present laundry care compositions may comprise polymeric or non-polymeric dyes, organic or inorganic pigments, or mixtures thereof. Preferably the hueing dye comprises a polymeric dye, comprising a chromophore constituent and a polymeric constituent. The chromophore constituent is characterized in that it absorbs light in the wavelength range of blue, red, violet, purple, or combinations thereof upon exposure to light. In one aspect, the chromophore constituent exhibits an absorbance spectrum maximum from about 520 nanometers to about 640 nanometers in water and/or methanol, and in another aspect, from about 560 nanometers to about 610 nanometers in water and/or methanol.

Although any suitable chromophore may be used, the dye chromophore is preferably selected from benzodifuranes, methine, triphenylmethanes, naphthalimides, pyrazole, naphthoquinone, anthraquinone, azo, oxazine, azine, xanthene, triphenodioxazine and phthalocyanine dye chromophores. Mono and di-azo dye chromophores are may be preferred.

The hueing dye may comprise a dye polymer comprising a chromophore covalently bound to one or more of at least three consecutive repeat units. It should be understood that the repeat units themselves do not need to comprise a chromophore. The dye polymer may comprise at least 5, or at least 10, or even at least 20 consecutive repeat units.

The repeat unit can be derived from an organic ester such as phenyl dicarboxylate in combination with an oxyalkyleneoxy and a polyoxyalkyleneoxy. Repeat units can be derived from alkenes, epoxides, aziridine, carbohydrate including the units that comprise modified celluloses such as hydroxyalkylcellulose; hydroxypropyl cellulose; hydroxypropyl methylcellulose; hydroxybutyl cellulose; and, hydroxybutyl methylcellulose or mixtures thereof. The repeat units may be derived from alkenes, or epoxides or mixtures thereof. The repeat units may be  $C_2-C_4$  alkyleneoxy groups, sometimes called alkoxy groups, preferably derived from  $C_2-C_4$  alkylene oxide. The repeat units may be  $C_2-C_4$  alkoxy groups, preferably ethoxy groups.

For the purposes of the present invention, the at least three consecutive repeat units form a polymeric constituent. The polymeric constituent may be covalently bound to the chromophore group, directly or indirectly via a linking group. Examples of suitable polymeric constituents include polyoxyalkylene chains having multiple repeating units. In one aspect, the polymeric constituents include polyoxyalkylene chains having from 2 to about 30 repeating units, from 2 to about 20 repeating units, from 2 to about 10 repeating units or even from about 3 or 4 to about 6 repeating units. Non-limiting examples of polyoxyalkylene chains include ethylene oxide, propylene oxide, glycidol oxide, butylene oxide and mixtures thereof.

#### Surfactants—

The compositions according to the present invention may comprise a surfactant or surfactant system wherein the surfactant can be selected from nonionic surfactants, anionic surfactants, cationic surfactants, amphotolytic surfactants, zwitterionic surfactants, semi-polar nonionic surfactants and mixtures thereof.

The surfactant is typically present at a level of from about 0.01% to about 60%, from about 0.1% to about 60%, from about 1% to about 50% or even from about 5% to about 40% by weight of the subject composition. Alternatively, the surfactant may be present at a level of from about 0.01% to about 60%, from about 0.01% to about 50%, from about 0.01% to about 40%, from about 0.1% to about 25%, from about 1% to about 10%, by weight of the subject composition.

#### Chelating Agents—

The compositions herein may contain a chelating agent. Suitable chelating agents include copper, iron and/or manganese chelating agents and mixtures thereof. When a chelating agent is used, the composition may comprise from about 0.1% to about 15% or even from about 3.0% to about 10% chelating agent by weight of the subject composition.

#### Dye Transfer Inhibiting Agents—

The compositions of the present invention may also include one or more dye transfer inhibiting agents. Suitable polymeric dye transfer inhibiting agents include, but are not limited to, polyvinylpyrrolidone polymers, polyamine N-oxide polymers, copolymers of N-vinylpyrrolidone and N-vinylimidazole, polyvinyloxazolidones and polyvinylimidazoles or mixtures thereof.

When present in a subject composition, the dye transfer inhibiting agents may be present at levels from about 0.0001% to about 10%, from about 0.01% to about 5% or even from about 0.1% to about 3% by weight of the composition.

#### Dispersants—

The compositions of the present invention can also contain dispersants. Suitable water-soluble organic materials include the homo- or co-polymeric acids or their salts, in which the polycarboxylic acid comprises at least two carboxyl radicals separated from each other by not more than two carbon atoms.

#### Perfumes—

The dispersed phase may comprise a perfume that may include materials selected from the group consisting of perfumes such as 3-(4-t-butylphenyl)-2-methyl propanal, 3-(4-t-butylphenyl)-propanal, 3-(4-isopropylphenyl)-2-methylpropanal, 3-(3,4-methylenedioxyphenyl)-2-methylpropanal, and 2,6-dimethyl-5-heptenal, alpha-damascone, beta-damascone, gamma-damascone, beta-damascenone, 6,7-dihydro-1,1,2,3,3-pentamethyl-4(5H)-indanone, methyl-7,3-dihydro-2H-1,5-benzodioxepine-3-one, 2-[2-(4-methyl-3-cyclohexenyl-1-yl)propyl]cyclopentan-2-one, 2-sec-butylcyclohexanone, and beta-dihydro ionone, linalool, ethyllinalool, tetrahydrolinalool, and dihydromyrcenol.

#### Perfume Delivery Technologies—

The fluid fabric enhancer compositions may comprise one or more perfume delivery technologies that stabilize and enhance the deposition and release of perfume ingredients from treated substrate. Such perfume delivery technologies can also be used to increase the longevity of perfume release from the treated substrate. Perfume delivery technologies, methods of making certain perfume delivery technologies and the uses of such perfume delivery technologies are disclosed in US 2007/0275866 A1.

In one aspect, the fluid fabric enhancer composition may comprise from about 0.001% to about 20%, or from about 0.01% to about 10%, or from about 0.05% to about 5%, or even from about 0.1% to about 0.5% by weight of the perfume delivery technology. In one aspect, said perfume delivery technologies may be selected from the group consisting of: perfume microcapsules, pro-perfumes, polymer particles, functionalized silicones, polymer assisted deliv-

ery, molecule assisted delivery, fiber assisted delivery, amine assisted delivery, cyclodextrins, starch encapsulated accord, zeolite and inorganic carrier, and mixtures thereof:

In one aspect, said perfume delivery technology may comprise microcapsules formed by at least partially surrounding a benefit agent with a wall material. Said benefit agent may include materials selected from the group consisting of perfumes such as 3-(4-t-butylphenyl)-2-methyl propanal, 3-(4-t-butylphenyl)-propanal, 3-(4-isopropylphenyl)-2-methylpropanal, 3-(3,4-methylenedioxyphenyl)-2-methylpropanal, and 2,6-dimethyl-5-heptenal,  $\alpha$ -damascone,  $\beta$ -damascone,  $\delta$ -damascone,  $\beta$ -damascenone, 6,7-dihydro-1,1,2,3,3-pentamethyl-4(5H)-indanone, methyl-7,3-dihydro-2H-1,5-benzodioxepine-3-one, 2-[2-(4-methyl-3-cyclohexenyl-1-yl)propyl]cyclopentan-2-one, 2-sec-butylcyclohexanone, and  $\beta$ -dihydro ionone, linalool, ethyllinalool, tetrahydrolinalool, and dihydromyrcenol; silicone oils, waxes such as polyethylene waxes; essential oils such as fish oils, jasmine, camphor, lavender; skin coolants such as menthol, methyl lactate; vitamins such as Vitamin A and E; sunscreens; glycerine; catalysts such as manganese catalysts or bleach catalysts; bleach particles such as perborates; silicon dioxide particles; antiperspirant actives; cationic polymers and mixtures thereof. Suitable benefit agents can be obtained from Givaudan Corp. of Mount Olive, N.J., USA, International Flavors & Fragrances Corp. of South Brunswick, N.J., USA, or Firmenich Company of Geneva, Switzerland. In one aspect, the microcapsule wall material may comprise: melamine, polyacrylamide, silicones, silica, polystyrene, polyurea, polyurethanes, polyacrylate based materials, gelatin, styrene malic anhydride, polyamides, and mixtures thereof. In one aspect, said melamine wall material may comprise melamine cross-linked with formaldehyde, melamine-dimethoxyethanol crosslinked with formaldehyde, and mixtures thereof. In one aspect, said polystyrene wall material may comprise polystyrene cross-linked with divinylbenzene. In one aspect, said polyurea wall material may comprise urea crosslinked with formaldehyde, urea crosslinked with gluteraldehyde, and mixtures thereof. In one aspect, said polyacrylate based materials may comprise polyacrylate formed from methylmethacrylate/dimethylaminomethyl methacrylate, polyacrylate formed from amine acrylate and/or methacrylate and strong acid, polyacrylate formed from carboxylic acid acrylate and/or methacrylate monomer and strong base, polyacrylate formed from an amine acrylate and/or methacrylate monomer and a carboxylic acid acrylate and/or carboxylic acid methacrylate monomer, and mixtures thereof. In one aspect, the perfume microcapsule may be coated with a deposition aid, a cationic polymer, a non-ionic polymer, an anionic polymer, or mixtures thereof. Suitable polymers may be selected from the group consisting of: polyvinylformaldehyde, partially hydroxylated polyvinylformaldehyde, polyvinylamine, polyethyleneimine, ethoxylated polyethyleneimine, polyvinylalcohol, polyacrylates, and combinations thereof. In one aspect, one or more types of microcapsules, for example two microcapsules types having different perfume benefit agents may be used.

In one aspect, said perfume delivery technology may comprise an amine reaction product (ARP) or a thiol reaction product. One may also use "reactive" polymeric amines and or polymeric thiols in which the amine and/or thiol functionality is pre-reacted with one or more PRMs to form a reaction product. Typically the reactive amines are primary and/or secondary amines, and may be part of a polymer or a monomer (non-polymer). Such ARPs may also be mixed with additional PRMs to provide benefits of polymer-as-

sisted delivery and/or amine-assisted delivery. Nonlimiting examples of polymeric amines include polymers based on polyalkylimines, such as polyethyleneimine (PEI), or polyvinylamine (PVAm). Nonlimiting examples of monomeric (non-polymeric) amines include hydroxyl amines, such as 2-aminoethanol and its alkyl substituted derivatives, and aromatic amines such as anthranilates. The ARPs may be premixed with perfume or added separately in leave-on or rinse-off applications. In another aspect, a material that contains a heteroatom other than nitrogen and/or sulfur, for example oxygen, phosphorus or selenium, may be used as an alternative to amine compounds. In yet another aspect, the aforementioned alternative compounds can be used in combination with amine compounds. In yet another aspect, a single molecule may comprise an amine moiety and one or more of the alternative heteroatom moieties, for example, thiols, phosphines and selenols. The benefit may include improved delivery of perfume as well as controlled perfume release. Suitable ARPs as well as methods of making same can be found in USPA 2005/0003980 A1 and U.S. Pat. No. 6,413,920 B1.

#### Processes of Making Products

The compositions of the present invention can be formulated into any suitable form and prepared by any process chosen by the formulator, non-limiting examples of which are described in Applicants' examples and in US 2013/0109612 A1 which is incorporated herein by reference.

In one aspect, the compositions disclosed herein may be prepared by combining the components thereof in any convenient order and by mixing, e.g., agitating, the resulting component combination to form a phase stable fabric and/or home care composition. In one aspect, a fluid matrix may be formed containing at least a major proportion, or even substantially all, of the fluid components with the fluid components being thoroughly admixed by imparting shear agitation to this liquid combination. For example, rapid stirring with a mechanical stirrer may be employed.

#### Method of Use

The compositions of the present invention may be used in any conventional manner. In short, they may be used in the same manner as products that are designed and produced by conventional methods and processes. For example, compositions of the present invention can be used to treat a *situs inter alia* a surface or fabric. Typically at least a portion of the *situs* is contacted with an aspect of Applicants' composition, in neat form or diluted in a wash liquor, and then the *situs* is optionally washed and/or rinsed. For purposes of the present invention, washing includes but is not limited to, scrubbing, and mechanical agitation. The fabric may comprise any fabric capable of being laundered in normal consumer use conditions. When the wash solvent is water, the water temperature typically ranges from about 5° C. to about 90° C. and, when the *situs* comprises a fabric, the water to fabric mass ratio is typically from about 1:1 to about 100:1.

The consumer products of the present invention may be used as liquid fabric enhancers wherein they are applied to a fabric and the fabric is then dried via line drying and/or drying in an automatic dryer.

In one aspect, a liquor that comprises a sufficient amount of a composition that comprises a fabric softener active, a silicone polymer and a cationic polymer, to satisfy the following equation:

$$[(a)+(b)+(c)]w=z$$

wherein, a is a weight percent of fabric softener active other than silicone polymer in said composition, preferably

a is from about 0 to about 20 weight percent, more preferably a is from about 1 to about 15 weight percent, more preferably a is from about 3 to about 10 weight percent, most preferably a is from about 7 to about 10 weight percent; b is the weight percent silicone polymer in said composition, preferably b is from about 0 to about 10 weight percent, more preferably b is from about 0.5 to about 5 weight percent, most preferably b is from about 1 to about 3 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; x is a number from about 1 to about 5, preferably x is a number about 2; y is a number from about 1 to about 10, preferably y is a number about 2; z is a number from about 1 to about 10, preferably z is a number from about 1 to about 7, more preferably, z is a number from about 2 to about 4. Preferably, said composition that comprises a fabric softener active, a silicone polymer and a cationic polymer is a composition disclosed and/or claimed in this specification. In one aspect, said liquor may comprise an anionic surfactant, preferably 1 ppm to 1000 ppm, more preferably 1 ppm to 100 ppm of an anionic surfactant. Preferably for said liquor, a divided by b is a number from about 0.5 to about 10, preferably a divided by b is a number from about 1 to about 10, more preferably a divided by b is a number from about 1 to about 4, most preferably a divided by b is a number from about 2 to about 3.

In one aspect, a method of treating a fabric comprising optionally washing, rinsing and/or drying a fabric then contacting said fabric with a liquor that comprises a sufficient amount of a composition that comprises a fabric softener active, a silicone polymer and a cationic polymer, to satisfy the following equation:

$$[(a)+(b)+(c)]w=z$$

wherein, a is a weight percent of fabric softener active other than silicone polymer in said composition, preferably a is from about 0 to about 20 weight percent, more preferably a is from about 1 to about 15 weight percent, more preferably a is from about 3 to about 10 weight percent, most preferably a is from about 7 to about 10 weight percent; b is the weight percent silicone polymer in said composition, preferably b is from about 0 to about 10 weight percent, more preferably b is from about 0.5 to about 5 weight percent, most preferably b is from about 1 to about 3 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; x is a number from about 1 to about 5, preferably x is a number about 2; y is a number from about 1 to about 10, preferably y is a number from about 1 to about 5, more preferably y is a number about 2; z is a number from about 1 to about 10, preferably z is a number from about 1 to about 7, more preferably, z is a number from about 2 to about 4. Preferably, said composi-

tion that comprises a fabric softener active, a silicone polymer and a cationic polymer is a composition disclosed and/or claimed in this specification. In one aspect, said liquor may comprise an anionic surfactant, preferably 1 ppm to 1000 ppm, more preferably 1 ppm to 100 ppm of an anionic surfactant. Preferably for said method, a divided by b is a number from about 0.5 to about 10, preferably a divided by b is a number from about 1 to about 10, more preferably a divided by b is a number from about 1 to about 4, most preferably a divided by b is a number from about 2 to about 3.

In one aspect, a method of treating a fabric comprising optionally washing, rinsing and/or drying a fabric then contacting said fabric with a liquor that comprises a sufficient amount of a composition that comprises a fabric softener active and a cationic polymer, to satisfy the following equation:

$$[(a+y(c))w=z]$$

wherein, a is a weight percent fabric softener active in said composition, preferably a is from about 0 to about 20 weight percent, more preferably a is from about 1 to about 15 weight percent, more preferably a is from about 3 to about 10 weight percent, most preferably a is from about 7 to about 10 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; y is a number from about 1 to about 10, preferably y is a number from about 1 to about 5, more preferably y is a number about 2; z is a number from about 1 to about 10, preferably z is a number from about 1 to about 7, more preferably, z is a number from about 2 to about 4. Preferably, said composition that comprises a fabric softener active and a cationic polymer is a composition disclosed and/or claimed in this specification. In one aspect, said liquor may comprise an anionic surfactant, preferably 1 ppm to 1000 ppm, more preferably 1 ppm to 100 ppm of an anionic surfactant.

In one aspect, a liquor that comprises a sufficient amount of a composition that comprises a fabric softener active and a cationic polymer, to satisfy the following equation:

$$[(a+y(c))w=z]$$

wherein, a is a weight percent fabric softener active in said composition, preferably a is from about 0 to about 20 weight percent, more preferably a is from about 1 to about 15 weight percent, more preferably a is from about 3 to about 10 weight percent, most preferably a is from about 7 to about 10 weight percent; c is the weight percent of cationic polymer in said composition, preferably c is from about 0.01 to about 5 weight percent, more preferably c is from about 0.01 to about 1 weight percent, most preferably c is from about 0.03 to about 0.5 weight percent; wherein said weight percentages are, for purposes of said equation, converted to decimal values; w is the dose in grams divided by 1 gram, preferably w is a number from about 10 to about 45, more preferably w is a number from about 15 to about 40; y is a number from about 1 to about 10, preferably y is a number from about 1 to about 5, more preferably y is a number about 2; z is a number from about 1 to about 10, preferably z is a number from about 1 to about 7, more

preferably, z is a number from about 2 to about 4. Preferably, said composition that comprises a fabric softener active and a cationic polymer is a composition. In one aspect, said liquor may comprise an anionic surfactant, preferably 1 ppm to 1000 ppm, more preferably 1 ppm to 100 ppm of an anionic surfactant.

#### Test Methods

##### 10 Viscosity Slope Method 1

The viscosity slope value quantifies the rate at which the viscosity increases as a function of increasing polymer concentration. The viscosity slope of a single polymer or of a dual polymer system is determined from viscosity measurements conducted on a series of aqueous solutions which span a range of polymer concentrations. The viscosity slope of a polymer is determined from a series of aqueous polymer solutions and which are termed polymer solvent solutions. The aqueous phase is prepared gravimetrically by adding hydrochloric acid to deionized water to reach a pH of about 3.0. A series of polymer solvent solutions are prepared to logarithmically span between 0.01 and 1 weight percent of the polymer in the aqueous phase. Each polymer solvent solutions is prepared gravimetrically by mixing the polymer and solvent with a SpeedMixer DAC 150 FVZ-K (made by FlackTek Inc. of Landrum, S.C.) for 1 minute at 2,500 RPM in a Max 60 cup or Max 100 cup to the target polymer weight percent of the polymer solvent solution. Polymer solvent solutions are allowed to come to equilibrium by resting for at least 24 hours. Viscosity as a function of shear rate of each polymer solvent solutions is measured at 40 different shear rates using an Anton Paar Rheometer with a DSR 301 measuring head and concentric cylinder geometry. The time differential for each measurement is logarithmic over the range of 180 and 10 seconds and the shear rate range for the measurements is 0.001 to 500 1/seconds (measurements taken from the low shear rate to the high shear rate).

Viscosity at a shear rate of 0.01 1/seconds as a function of polymer weight percent of the polymer solvent solution is fit using the equation  $Y=bX^a$  wherein X is the polymer concentration in the solvent polymer solution, Y is the polymer solvent solution viscosity, b is the extrapolated solvent polymer solution viscosity when X is extrapolated to unity and the exponent a is polymer concentration viscosity scaling power over the polymer concentration range where the exponent a is the highest value.

##### Viscosity Slope Method 2

The viscosity slope value quantifies the rate at which the viscosity increases as a function of increasing polymer concentration. The viscosity slope of a single polymer or of a dual polymer system is determined from viscosity measurements conducted on a series of aqueous solutions which span a range of polymer concentrations and which are termed polymer solvent solutions. Viscosity analyses are conducted using an Anton Paar Dynamic Shear Rheometer model DSR 301 Measuring Head, equipped with a 32-place Automatic Sample Changer (ASC) with reusable metal concentric cylinder geometry sample holders, and Rheoplus software version 3.62 (all from Anton Paar GmbH, Graz, Austria). All polymer solutions are mixed using a high-speed motorized mixer, such as a Dual Asymmetric Centrifuge SpeedMixer model DAC 150 FVZ-K (FlackTek Inc., Landrum, S.C., USA) or equivalent. The aqueous phase diluent for all of the aqueous polymer solutions is prepared by adding sufficient concentrated hydrochloric acid (e.g. 16 Baume, or 23% HCl) to deionized

water until a pH of about 3.0 is achieved. The polymer(s) are combined with the aqueous phase diluent in a mixer cup (such as the Flacktek Speedmixer Max 100 or Max 60) that is compatible with the mixer to be used and is of a suitable size to hold a sample volume of 35 mL to 100 mL. Sufficient polymer is added to the aqueous phase diluent to achieve a concentration of between 8000-10000 ppm of the single polymer, or of the polymer 2 in the case of a dual polymer system, and to yield a volume of between 35 mL to 100 mL. The mixture of the polymer(s) and the aqueous phase is mixed for 4 minutes at a speed of 3500 RPM. After mixing, this initial polymer solvent solution is put aside to rest in a sealed container for at least 24 hours.

A single viscosity measurement is obtained from each of 32 polymer solvent solutions wherein each solution has a different concentration of polymer. These 32 polymer solvent solutions comprise a series of solutions that span the concentration range of 1000 ppm to 4000 ppm, with the solutions spaced at concentration intervals of approximately every 100 ppm. Each of the 32 polymer solvent solution concentrations is prepared gravimetrically by mixing the initial 8000-10000 ppm polymer solvent solution with sufficient additional aqueous phase diluent to result in a solution having the required target concentration and a volume of 35 mL to 100 mL, which is then mixed for 2 minutes at a speed of 3500 RPM. All of the resultant polymer solvent solutions are put aside to rest in a sealed cup for at least 24 hours. Polymer solutions are loaded into the concentric cylinder sample holders of the rheometer's ASC, using a pipette to fill each cylinder up to the line indicating a volume of 23 mL. The samples are stored in the ASC of the rheometer at a temperature of approximately 21° C. for up to 36 hours until measured. The viscosity of each of the 32 polymer solvent solutions is measured at the shear rate of 0.0105 1/s, and the viscosity value in units of Pa·s is recorded as soon as the value being measured is stable and consistent. The recorded viscosity values measured at a shear rate of 0.0105 1/s are paired with the value of the respective concentration of the polymer solvent solution measured. The resultant paired data values are plotted as 32 data points on a graph with viscosity in units of Pa·s on the x-axis, and polymer concentration in units of ppm on the y-axis. This data set is subsampled repeatedly to yield 30 subsets, wherein each subset comprises three consecutive data points. The subset creation process begins with the data point at the lowest polymer concentration and advances in sequence increasing toward the highest polymer concentration, until 30 unique subsets have been created. The subset creation process advances up to higher concentrations in steps of 1 data point at a time.

The three data points in each subset are fit with the following linear equation, using linear least squares regression, to determine the value of the exponent "a" for each of the 30 subsets:

$$Y=bX^a$$

wherein;

X is the polymer concentration in the solvent polymer solution (in ppm),

Y is the polymer solvent solution viscosity (in Pa·s)

<sup>5</sup> b is the extrapolated solvent polymer solution viscosity (in Pa·s) when X is extrapolated to the value of 1 ppm, and the exponent a is a unitless parameter.

The Viscosity Slope value reported for the material being tested is the highest value calculated for the exponent "a", of all of the 30 values calculated for the exponent "a" from the <sup>10</sup> 30 subsets.

#### Brookfield Viscosity

<sup>15</sup> Brookfield viscosity is measured using a Brookfield DV-E viscometer. The liquid is contained in a glass jar, where the width of the glass jar is from about 5.5 to 6.5 cm and the height of the glass jar is from about 9 to about 11 cm. For viscosities below 500 cPs, use spindle LV2 at 60 RPM, and to measure viscosities from 500 to 2,000 cPs, use spindle LV3 at 60 RPM. The test is conducted in accordance with the <sup>20</sup> instrument's instructions. Initial Brookfield viscosity is defined as the Brookfield viscosity measured within 24 hours of making the subject composition.

#### Physical Stability

<sup>25</sup> Physical stability is assessed by visual observation of the product in an undisturbed glass jar, where the width of the glass jar is from about 5.5 to 6.5 cm and the height of the glass jar is from about 9 to about 11 cm, after 4 weeks at 25° C. Using a ruler with millimeter graduation, the height of the liquid in the jar and the height of any visually observed phase separation are measured. The Stability Index is defined as the height of the phase split divided by the height of the liquid in the glass jar. A product with no visually <sup>30</sup> observable phase split is given a stability index of zero.

## EXAMPLES

### Example 1

<sup>35</sup> Compositions having the listed amounts of materials are made by combining the ammonium quat active with water using shear then the other materials are combined with the ammonium quat/water and mixed to form a fabric softener composition. Adjunct ingredients such as perfume, dye and stabilizer may be added as desired.

|    | Silicone Active                                | Ammonium Quat Active                          | First Polymer*                                                | Second Polymer*                                |
|----|------------------------------------------------|-----------------------------------------------|---------------------------------------------------------------|------------------------------------------------|
| 45 | 0-0.5%;<br>0-5.0%;<br>1.0-3.0%; or<br>1.5-2.5% | 1 - 18%;<br>2 - 14%;<br>7 - 10%; or<br>4 - 8% | 0.01-0.50%;<br>0.02-0.20%;<br>0.03-0.15%;<br>or<br>0.04-0.12% | 0.01-0.35%;<br>0.02-0.15%;<br>or<br>0.03-0.12% |
| 50 |                                                |                                               |                                                               |                                                |

<sup>55</sup>\*As described in the present specification.

### Example 2

#### Fabric Softener Products

| (% wt)                      | F1   | F2  | F3   | F4   | F5  | F6  |
|-----------------------------|------|-----|------|------|-----|-----|
| FSA <sup>a</sup>            | 11.2 | 7   | 9    | —    | —   | —   |
| FSA <sup>b</sup>            | —    | —   | —    | —    | —   | 6   |
| FSA <sup>c</sup>            | —    | —   | —    | 14.5 | 13  | —   |
| Coco oil                    | 0.6  | 0.5 | 0.45 | —    | —   | —   |
| Low MW Alcohol <sup>d</sup> | 1.11 | 0.7 | 0.9  | 1.5  | 1.3 | 0.5 |
| Perfume                     | 1.75 | 0.6 | 2.1  | 1.5  | 2   | 1.2 |

|                                         |         |         |         |         |         |         |
|-----------------------------------------|---------|---------|---------|---------|---------|---------|
| Perfume encapsulate <sup>e</sup>        | 0.19    | 0.6     | 0.5     | 0.25    | 0.6     | 0.4     |
| Calcium Chloride(ppm)                   | 0.06    | 0.03    | 0.025   | 0.12    | 0.06    | —       |
| Chelant <sup>f</sup>                    | 0.005   | 0.005   | 0.005   | 0.005   | 0.005   | 0.006   |
| Preservative <sup>g</sup>               | 0.04    | 0.04    | 0.02    | 0.04    | 0.03    | 0.05    |
| Acidulent (Formic Acid)                 | 0.051   | 0.03    | 0.04    | 0.02    | 0.03    | —       |
| Antifoam <sup>h</sup>                   |         |         |         |         |         | 0.05    |
| Polymer 1 <sup>i</sup>                  | 0.17    | 0.15    | 0.2     | 0.12    | 0.16    | 0.35    |
| Polymer 2 <sup>i</sup>                  | 0.03    | 0.05    | 0.1     | 0.03    | 0.5     | 0.1     |
| Water soluble dialkyl quat <sup>j</sup> | 0.25    | 0.2     | 0.1     | 0.5     | —       | 0.25    |
| Dispersant <sup>k</sup>                 | —       | —       | —       | —       | —       | —       |
| Stabilizing Surfactant <sup>l</sup>     | —       | —       | —       | —       | —       | 0.1     |
| PDMS emulsion <sup>m</sup>              | —       | —       | 0.5     | —       | 2       | —       |
| Amino-functional Organosiloxane         | 3       | 2       |         | 1       | —       | —       |
| Polymer                                 |         |         |         |         |         |         |
| Dye (ppm)                               | 0.03    | 0.03    | 0.02    | 0.04    | 0.04    | 0.02    |
| Hydrochloric Acid                       | 0.0075  | 0.0075  | 0.008   | 0.01    | 0.01    | 0.01    |
| Deionized Water                         | Balance | Balance | Balance | Balance | Balance | Balance |

|                                         |         |         |         |         |         |         |
|-----------------------------------------|---------|---------|---------|---------|---------|---------|
| (% wt)                                  | F7      | F8      | F9      | F10     | F11     | F12     |
| FSA <sup>a</sup>                        | 12      | 9.5     | 8       | 6.5     | 5.3     | 2.5     |
| FSA <sup>b</sup>                        | —       | —       | —       | —       | —       | —       |
| FSA <sup>c</sup>                        | —       | —       | —       | —       | —       | —       |
| Coco oil                                | 0.6     | 0.475   | 0.4     | 0.325   | 0.265   | 0.125   |
| Low MW Alcohol <sup>d</sup>             | 0.9     | 1.11    | 0.95    | 1.05    | 0.78    | 0.35    |
| Perfume                                 | 3       | 1.41    | 1.00    | 0.55    | 1.55    | 1       |
| Perfume encapsulate <sup>e</sup>        | 0.6     | 0.15    | 0.25    | 0.62    | 0.98    | 0.25    |
| Calcium Chloride(ppm)                   | 0.07    | 0.23    | 0.16    | —       | —       | —       |
| Chelant <sup>f</sup>                    | 0.005   | 0.01    | 0.01    | 0.01    | 0.01    | 0.01    |
| Preservative <sup>g</sup>               | 0.04    | —       | —       | —       | —       | —       |
| Acidulent (Formic Acid)                 | 0.05    | 0.06    | 0.06    | 0.06    | 0.06    | —       |
| Antifoam <sup>h</sup>                   | —       | —       | —       | —       | —       | —       |
| Polymer 1 <sup>i</sup>                  | 0.14    | 0.08    | 0.12    | 0.06    | 0.04    | 0.08    |
| Polymer 2 <sup>i</sup>                  | 0.1     | 0.12    | 0.12    | 0.08    | 0.04    | —       |
| Water soluble dialkyl quat <sup>j</sup> | 0.35    | 0.11    | 0.11    | —       | 0.52    | 0.1     |
| Dispersant <sup>k</sup>                 | —       | —       | —       | —       | —       | —       |
| Stabilizing Surfactant <sup>l</sup>     | —       | —       | —       | —       | —       | —       |
| PDMS emulsion <sup>m</sup>              | 2       | —       | —       | —       | —       | 3       |
| Amino-functional Organosiloxane         | —       | —       | —       | —       | —       | —       |
| Polymer                                 |         |         |         |         |         |         |
| Dye (ppm)                               | 0.02    | 0.03    | 0.03    | 0.03    | 0.03    | 0.02    |
| Hydrochloric Acid                       | 0.005   | 0.03    | 0.03    | 0.03    | 0.03    | 0.02    |
| Deionized Water                         | Balance | Balance | Balance | Balance | Balance | Balance |

|                                         |         |         |         |         |         |         |
|-----------------------------------------|---------|---------|---------|---------|---------|---------|
| (% wt)                                  | F13     | F14     | F15     | F16     | F17     | F18     |
| FSA <sup>a</sup>                        | 14.7    | 14.7    | 11.1    | 9.5     | 6.25    | 5.1     |
| FSA <sup>b</sup>                        | —       | —       | —       | —       | —       | —       |
| FSA <sup>c</sup>                        | —       | —       | —       | —       | —       | —       |
| Coco oil                                | 0.735   | 0.735   | 0.555   | 0.475   | 0.3125  | 0.255   |
| Low MW Alcohol <sup>d</sup>             | 0.88    | 0.58    | 0.45    | 0.52    | 0.33    | 0.22    |
| Perfume                                 | 1.65    | 1.65    | 1.65    | 1.4     | 3.12    | 0.65    |
| Perfume encapsulate <sup>e</sup>        | 0.26    | 0.26    | 0.26    | 0.43    | 0.26    | 0.75    |
| Calcium Chloride(ppm)                   | 0.23    | 0.23    | —       | 0.23    | 0.23    | 0.23    |
| Chelant <sup>f</sup>                    | 0.01    | 0.01    | 0.01    | 0.01    | 0.01    | 0.01    |
| Preservative <sup>g</sup>               | —       | 0.001   | —       | 0.001   | 0.001   | 0.001   |
| Acidulent (Formic Acid)                 | 0.06    | —       | —       | —       | —       | —       |
| Antifoam <sup>h</sup>                   | —       | —       | —       | —       | —       | —       |
| Polymer 1 <sup>i</sup>                  | 0.07    | 0.07    | 0.05    | 0.06    | 0.06    | 0.06    |
| Polymer 2 <sup>i</sup>                  | 0.09    | 0.09    | 0.05    | 0.09    | 0.09    | 0.09    |
| Water soluble dialkyl quat <sup>j</sup> | —       | 0.29    | 0.29    | 0.29    | 0.29    | 0.29    |
| Dispersant <sup>k</sup>                 | —       | —       | —       | —       | —       | —       |
| Stabilizing Surfactant <sup>l</sup>     | —       | —       | —       | —       | —       | —       |
| PDMS emulsion <sup>m</sup>              | —       | 1.12    | —       | —       | —       | —       |
| Amino-functional Organosiloxane         | —       | —       | 1.8     | 2.2     | 3.1     | 1.8     |
| Polymer                                 |         |         |         |         |         |         |
| Dye (ppm)                               | 0.03    | 0.03    | 0.03    | 0.03    | 0.03    | 0.03    |
| Hydrochloric Acid                       | 0.03    | 0.03    | 0.03    | 0.03    | 0.03    | 0.03    |
| Deionized Water                         | Balance | Balance | Balance | Balance | Balance | Balance |

|                                  |       |        |      |      |      |      |
|----------------------------------|-------|--------|------|------|------|------|
| (% wt)                           | F19   | F20    | F21  | F22  | F23  | F24  |
| FSA <sup>a</sup>                 | 14.7  | 6.25   | 10.2 | 5    | 11   | 15   |
| FSA <sup>b</sup>                 | —     | —      | —    | —    | —    | —    |
| FSA <sup>c</sup>                 | —     | —      | —    | —    | —    | —    |
| Coco oil                         | 0.735 | 0.3125 | 0.51 | 0.3  | 0.6  | 0.8  |
| Low MW Alcohol <sup>d</sup>      | 0.58  | 0.11   | 0.58 | 0.95 | 0.95 | 0.95 |
| Perfume                          | 1.65  | 0.35   | 1.65 | 1.00 | 1.00 | 1.00 |
| Perfume encapsulate <sup>e</sup> | 0.26  | 1.33   | 0.26 | 0.25 | 0.25 | 0.25 |

|                                         |         |         |         |         |         |         |
|-----------------------------------------|---------|---------|---------|---------|---------|---------|
| Calcium Chloride(ppm)                   | 0.23    | 0.42    | 0.23    | 0.16    | 0.16    | 0.16    |
| Chelant <sup>f</sup>                    | 0.01    | 0.01    | 0.01    | 0.01    | 0.01    | 0.01    |
| Preservative <sup>g</sup>               | 0.001   | —       | 0.001   | —       | —       | —       |
| Acidulent (Formic Acid)                 | —       | 0.06    | —       | 0.06    | 0.06    | 0.06    |
| Antifoam <sup>h</sup>                   | —       | 0.02    | —       | —       | —       | —       |
| Polymer 1 <sup>i</sup>                  | 0.03    | 0.25    | 0.01    | 0.12    | 0.12    | 0.12    |
| Polymer 2 <sup>i</sup>                  | 0.04    | 0.18    | 0.02    | 0.12    | 0.12    | 0.12    |
| Water soluble dialkyl quat <sup>j</sup> | 0.29    | 0.29    | 0.29    | 0.11    | 0.11    | 0.11    |
| Dispersant <sup>k</sup>                 | —       | —       | 0.15    | —       | —       | —       |
| Stabilizing Surfactant <sup>l</sup>     | —       | —       | 0.45    | —       | —       | —       |
| PDMS emulsion <sup>m</sup>              | 1.12    | —       | 0.85    | —       | —       | —       |
| Amino-functional Organosiloxane Polymer | —       | 3.1     | 0.95    | —       | —       | —       |
| Dye (ppm)                               | 0.03    | 0.03    | —       | 0.03    | 0.03    | 0.03    |
| Hydrochloric Acid                       | 0.03    | 0.03    | 0.03    | 0.03    | 0.03    | 0.03    |
| Deionized Water                         | Balance | Balance | Balance | Balance | Balance | Balance |

<sup>a</sup>N,N-di(alkanoyloxyethyl)-N,N-dimethylammonium chloride where alkyl consists predominantly of C<sub>16</sub>-C<sub>18</sub> alkyl chains with an IV value of about 20 available from Evonik

<sup>b</sup>Methyl bis[ethyl (tallowate)-2-hydroxyethyl ammonium methyl sulfate available from Stepan

<sup>c</sup>N,N-di(alkanoyloxyethyl)-N,N-dimethylammonium chloride where alkyl consists predominantly of C<sub>16</sub>-C<sub>18</sub> alkyl chains with an IV value of about 52 available from Evonik

<sup>d</sup>Low molecular weight alcohol such as ethanol or isopropanol

<sup>e</sup>Perfume microcapsules available ex Appleton Papers, Inc.

<sup>f</sup>Diethylenetriaminepentaacetic acid or hydroxyl ethylidene-1,1-diphosphonic acid

<sup>g</sup>1,2-Benzisothiazolin-3-ONE (BIT) under the trade name Proxel available from Lonza

<sup>h</sup>Silicone antifoam agent available from Dow Corning ® under the trade name DC2310

<sup>i</sup>Polymer 1 and Polymer 2 are chosen such that one polymer is synthetic and the other polymer is bio-derived. Such polymers are described as First Polymer and Second Polymer in the present specification.

<sup>j</sup>Didecyl dimethyl ammonium chloride under the trade name Bardac ® 2280 or Hydrogenated tallowalkyl(2-ethylhexyl)dimethyl ammonium methylsulfate from AkzoNobel under the tradename Arquad ® HTL8-MS

<sup>k</sup>Non-ionic surfactant from BASF under the trade name Lutensol ® XL-70

<sup>l</sup>Non-ionic surfactant, such as TWEEN 20™ or TAE80 (tallow ethoxylated alcohol, with average degree of ethoxylation of 80)

<sup>m</sup>Polydimethylsiloxane emulsion from Dow Corning under the trade name DC346 ®.

### Example 3

#### Fabric Preparation Example

Fabrics are assessed using Kenmore FS 600 and/or 80 series washer machines. Wash Machines are set at: 32° C./15° C. wash/rinse temperature, 6 gpg hardness, normal cycle, and medium load (64 liters). Fabric bundles consist of 2.5 kilograms of clean fabric consisting of 100% cotton. Test swatches are included with this bundle and comprise of 100% cotton Euro Touch terrycloth towels (purchased from Standard Textile, Inc. Cincinnati, Ohio). Prior to treatment with any test products, the fabric bundles are stripped according to the Fabric Preparation-Stripping and Desizing procedure before running the test. Tide Free liquid detergent (1x recommended dose) is added under the surface of the water after the machine is at least half full. Once the water stops flowing and the washer begins to agitate, the clean fabric bundle is added. When the machine is almost full with rinse water, and before agitation has begun, the fabric care testing composition is slowly added (1x dose), ensuring that none of the fabric care testing composition comes in direct contact with the test swatches or fabric bundle. When the wash/rinse cycle is complete, each wet fabric bundle is transferred to a corresponding dryer. The dryer used is a Maytag commercial series (or equivalent) electric dryer, with the timer set for 55 minutes on the cotton/high heat/timed dry setting. This process is repeated for a total of three (3) complete wash-dry cycles. After the third drying cycle and once the dryer stops, 12 Terry towels from each fabric bundle are removed for actives deposition analysis. The fabrics are then placed in a constant Temperature/Relative Humidity (21° C., 50% relative humidity) controlled grading room for 12-24 hours and then graded for softness and/or actives deposition.

The Fabric Preparation-Stripping and Desizing procedure includes washing the clean fabric bundle (2.5 Kg of fabric

30 comprising 100% cotton) including the test swatches of 100% cotton EuroTouch terrycloth towels for 5 consecutive wash cycles followed by a drying cycle. AATCC (American Association of Textile Chemists and Colorists) High Efficiency (HE) liquid detergent is used to strip/de-size the test 35 swatch fabrics and clean fabric bundle (1x recommended dose per wash cycle). The wash conditions are as follows: Kenmore FS 600 and/or 80 series wash machines (or equivalent), set at: 48° C./48° C. wash/rinse temperature, water 40 hardness equal to 0 gpg, normal wash cycle, and medium sized load (64 liters). The dryer timer is set for 55 minutes on the cotton/high/timed dry setting.

### Example 4

#### Silicone on Fabric Measurement Method

Silicone is extracted from approximately 0.5 grams of 50 fabric (previously treated according to the test swatch treatment procedure) with 12 mL of either 50:50 toluene:methylisobutyl ketone or 15:85 ethanol:methylisobutyl ketone in 55 20 mL scintillation vials. The vials are agitated on a pulsed vortexer for 30 minutes. The silicone in the extract is quantified using inductively coupled plasma optical emission spectrometry (ICP-OES). ICP calibration standards of known silicone concentration are made using the same or a 60 structurally comparable type of silicone raw material as the products being tested. The working range of the method is 8-2300 µg silicone per gram of fabric. Concentrations greater than 2300 µg silicone per gram of fabric can be 65 assessed by subsequent dilution. Deposition efficiency index of silicone is determined by calculating as a percentage, how much silicone is recovered, via the aforementioned extraction and measurement technique, versus how much is delivered via the formulation examples. The analysis is performed on terrycloth towels (EuroSoft towel, sourced from

41

Standard Textile, Inc, Cincinnati, Ohio) that are treated according to the wash procedure outlined herein.

## Example 5

## Example for Determining the Recovery Index for Organo Siloxane Polymer

The Recovery Index is measured using a Tensile and Compression Tester Instrument, such as the Instron Model 5565 (Instron Corp., Norwood, Mass., U.S.A.). The instrument is configured by selecting the following settings: the mode is Tensile Extension; the Waveform Shape is Triangle; the Maximum Strain is 10%, the Rate is 0.83 mm/sec, the number of Cycles is 4; and the Hold time is 15 seconds between cycles.

- 1) Determine the weight of one approximately 25.4 cm square swatch of 100% cotton woven fabric, (a suitable fabric is the Mercerized Combed Cotton Warp Sateen, Product Code 479, available from Testfabrics Inc., West Pittston, Pa., USA).
- 2) Determine the amount of organo siloxane polymer required to deposit 5 mg of the polymer per gram of fabric swatch and weigh that amount into a 50 ml plastic centrifuge tube with a lid.
- 3) Dilute the organo siloxane polymer to 1.3 times the weight of the swatch with a solvent that completely dissolves or disperses the organo siloxane polymer (examples: isopropyl alcohol, THF, N,N-dimethylacetamide, water).
- 4) Thoroughly disperse or dissolve silicone polyurethane with shaking or vortex stirring as needed.
- 5) Place fabric swatch lying flat into a stainless steel tray that is larger than the swatch.
- 6) Pour the organo siloxane polymer solution over the entire swatch as evenly as possible.
- 7) Fold the swatch twice to quarter, then roll it up while gently squeezing to disperse solution to the entire swatch.
- 8) Unfold and repeat Step 7, folding in the opposite direction
- 9) To make a control swatch, repeat the procedure described above using 1.3× weight of solvent only (nil active).
- 10) Lay each swatch on a separate piece of aluminum foil and place in a fume hood to dry overnight.
- 11) Cure each swatch in an oven with appropriate ventilation at 90° C. for 5 minutes, (a suitable oven is the Mathis Labdryer, with 1500 rpm fan rotation) (Werner Mathis AG, Oberhasli, Switzerland).
- 12) Condition fabrics in a constant temperature (21° C.+/-2° C.) and humidity (50% RH+/-5% RH) room for at least 6 hours.
- 13) With scissors, cut the edge of one entire side of each swatch in the warp direction and carefully remove fabric threads one at a time without stressing the fabric until an even edge is achieved.
- 14) Cut 4 strips of fabric from each swatch (die or rotary cut), parallel to the even edge, that are 2.54 cm wide and at least 10 cm long
- 15) Evenly clamp the top and bottom (narrower edges) of the fabric strip into the 2.54 cm grips on the tensile tester instrument with a 2.54 cm gap setting, loading a small amount of force (0.1N-0.2N) on the sample.
- 16) Strain to 10% at 0.83 mm/s and return to 2.54 cm gap at the same rate.

42

- 17) Release bottom clamp and re-clamp sample during the hold cycle, loading 0.1N-0.2N of force on the sample.
- 18) Repeat Steps 15-16 until 4 hysteresis cycles have been completed for the sample.
- 19) Analyze 4 fabric samples per treatment swatch by the above method and average the tensile strain values recorded at 0.1N unload for Cycle 4. Recovery is calculated as follows:

$$\% \text{ Recovery} = \frac{(10 - \text{Tensile Strain at } 0.1N)}{10} \times 100$$

$$20) \text{ Recovery Index} = \frac{\% \text{ Recovery of Treatment}}{\% \text{ Recovery of Control}}$$

## Example 6

## Fabric Friction Measures Example

For the examples cited a Thwing-Albert FP2250 Friction/Peel Tester with a 2 kilogram force load cell is used to measure fabric to fabric friction. (Thwing Albert Instrument Company, West Berlin, N.J.). The sled is a clamping style sled with a 6.4 by 6.4 cm footprint and weighs 200 g (Thwing Albert Model Number 00225-218). A comparable instrument to measure fabric to fabric friction would be an instrument capable of measuring frictional properties of a horizontal surface. A 200 gram sled that has footprint of 6.4 cm by 6.4 cm and has a way to securely clamp the fabric without stretching it would be comparable. It is important, though, that the sled remains parallel to and in contact with the fabric during the measurement. The distance between the load cell to the sled is set at 10.2 cm. The crosshead arm height to the sample stage is adjusted to 25 mm (measured from the bottom of the cross arm to the top of the stage) to ensure that the sled remains parallel to and in contact with the fabric during the measurement. The following settings are used to make the measure:

|                       |             |
|-----------------------|-------------|
| T2 (Kinetic Measure): | 10.0 sec    |
| Total Time:           | 20.0 sec    |
| Test Rate:            | 20.0 cm/min |

The 11.4 cm×6.4 cm cut fabric piece is attached to the clamping sled with the face down (so that the face of the fabric on the sled is pulled across the face of the fabric on the sample plate) which corresponds to friction sled cut. The loops of the fabric on the sled are oriented such that when the sled is pulled, the fabric is pulled against the nap of the loops of the test fabric cloth. The fabric from which the sled sample is cut is attached to the sample table such that the sled drags over the "Friction Drag Area". The loop orientation is such that when the sled is pulled over the fabric it is pulled against the loops.

The sled is placed on the fabric and attached to the load cell. The crosshead is moved until the load cell registers between ~1.0-2.0 gf, and is then moved back until the load reads 0.0 gf. At this point the sled drag is commenced and the Kinetic Coefficient of Friction (kCOF) recorded at least every second during the sled drag. The kinetic coefficient of friction is averaged over the time frame starting at 10 seconds and ending at 20 seconds for the sled speed set at 20.0 cm/min. For each treatment, at least ten replicate fabrics are measured.

## Perfume Release from Head Space Over Fabric Measurement Method

Fabrics were treated with compositions of the current invention using the Fabric Preparation method described within. The perfume release over fabric data was generated using standard dynamic purge and trap analysis of fabric headspace with gas chromatography (GC) and detector to measure perfume headspace levels. The headspace analysis was performed on wet and dry fabric and total perfume counts were normalized to one of the test legs to show the relative benefit of compositions of the present invention. For example, a wet fabric perfume headspace (normalized to 1.0) shows that Leg C has 50% more perfume headspace above the wet fabric than Leg A.

GC—Detector Analysis of Fabric Samples for Perfume Release: A total of 3 pieces of treated fabric 1"×2" in size are placed into 3 clean 40 ml bottles (for a total of 9 fabrics) and allowed to equilibrate for about 1 hour. The fabric pieces are cut from different fabrics within each load to account for fabric-to-fabric variability. Instrument conditions should be modified to achieve adequate PRM signal detection while avoiding peak saturation. A DB 5 column was used with 20 sec sample collection with a ramp of 40-180° C. at 5-10 deg/sec and a detector temperature of 35° C.

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm".

All documents cited in the Detailed Description of the Invention are, in relevant part, incorporated herein by reference; the citation of any document is not to be construed as an admission that it is prior art with respect to the present invention. To the extent that any meaning or definition of a term in this document conflicts with any meaning or definition of the same term in a document incorporated by reference, the meaning or definition assigned to the term in this written document shall govern.

While particular aspects of the present invention have been illustrated and described, it would be obvious to those skilled in the art that various other changes and modifications can be made without departing from the spirit and scope of the invention. It is therefore intended to cover in the appended claims all such changes and modifications that are within the scope of this invention.

What is claimed is:

1. A composition comprising, based upon total composition weight:

a) from about 0.01% to about 5% of a polymeric mixture that comprises a first polymer and a second polymer in a weight ratio of from about 1:1 to about 2:1; said first polymer being derived from the polymerization of from about 5 to 100 mole percent of a cationic vinyl addition monomer, from about 0 to 95 mole percent of a non-ionic vinyl addition monomer, from about 0 to about 50 mole percent of an anionic monomer, from about 50 ppm to 1,950 ppm of a cross-linking agent comprising two or more ethylenic functions, 0 ppm to about 10,000 ppm chain transfer agent,

wherein the cationic monomers are selected from the group consisting of methyl chloride quaternized

dimethyl aminoethylammonium acrylate, methyl chloride quaternized dimethyl aminoethylammonium methacrylate and mixtures thereof, and the non-ionic monomers are selected from the group consisting of acrylamide, dimethyl acrylamide and mixtures thereof, wherein the first polymer has the viscosity slope of greater than 3.7; said second polymer being derived from saccharides; and

10 b) from about 1% to about 35% of a fabric softener active; said composition being a fabric and home care product.

2. A composition according to claim 1, comprising from about 1% to about 35% of a fabric softener active selected from the group consisting of a quaternary ammonium compound, a silicone polymer, a polysaccharide, a clay, an amine, a fatty ester, a dispersible polyolefin, a polymer latex and mixtures thereof.

20 3. A composition according to claim 2, wherein;

a) said quaternary ammonium compound comprises an alkyl quaternary ammonium compound and mixtures thereof;

25 b) said silicone polymer is selected from the group consisting of cyclic silicones, polydimethylsiloxanes, aminosilicones, cationic silicones, silicone polyethers, silicone resins, silicone urethanes, and mixtures thereof;

c) said clay comprises a smectite clay;

30 d) said dispersible polyolefin is selected from the group consisting of polyethylene, polypropylene and mixtures thereof; and

e) said fatty ester is selected from the group consisting of a polyglycerol ester, a sucrose ester, a glycerol ester and mixtures thereof.

35 4. A composition according to claim 3, wherein said fabric softener active comprises a material selected from the group consisting of monoesterquats, diesterquats, triesterquats, and mixtures thereof.

40 5. A composition according to claim 2 wherein the fabric softening active has an Iodine Value of between 0-140, or when said fabric softening active comprises a partially hydrogenated fatty acid quaternary ammonium compound said fabric softening active has an Iodine Value of 25-60.

45 6. A composition according to claim 2, said composition comprising a quaternary ammonium compound and a silicone polymer.

7. A composition according to claim 2, said composition comprises, in addition to said fabric softener active, from about 0.001% to about 5% of a stabilizer that comprises an alkyl quaternary ammonium compound.

50 8. A composition according to claim 1, said composition having a Brookfield viscosity of from about 20 cps to about 1,000 cps.

55 9. A composition according to claim 1, said composition comprising an adjunct material selected from the group consisting of surfactants, builders, chelating agents, dye transfer inhibiting agents, dispersants, enzymes, and enzyme stabilizers, catalytic materials, bleach activators, hydrogen peroxide, sources of hydrogen peroxide, preformed peracids, polymeric dispersing agents, clay soil removal/anti-redeposition agents, brighteners, suds suppressors, dyes, hueing dyes, perfumes, perfume delivery systems, structure elasticizing agents, carriers, structurants, hydrotropes, processing aids, solvents and/or pigments and mixtures thereof.

60 10. A composition according to claim 9, said composition comprising perfume and/or a perfume delivery system.

65 11. A composition according to claim 1, said composition comprising one or more types of perfume microcapsules.

**45**

12. A composition according to claim 1, said composition having a pH from about 2 to about 4.

13. The composition of claim 1 wherein:

said first polymer is derived from the polymerization of from about 10 to 95 mole percent of a cationic vinyl addition monomer, from about 5 to 90 mole percent of a non-ionic vinyl addition monomer, from about 60 ppm to 1,900 ppm of a cross-linking agent comprising two or more ethylenic functions, with the proviso that said first polymer does not comprise an acrylamide unit; and

said second polymer is derived from starch, cellulose, and guar.

14. A composition according to claim 1, wherein said second polymer is derived from cationically modified saccharides and has a cationic charge density ranging from about 0.2 meq/gm to about 5 meq/gm, at the pH of intended use of the fabric softening composition.

**46**

15. A composition according to claim 1, wherein said second polymer is characterized by a Number Average Molecular Weight (Mn) from about 10,000 Daltons to about 500,000 Daltons.

16. A composition according to claim 1, wherein said anionic monomer is selected from the group consisting of acrylic acid, methacrylic acid, itaconic acid, crotonic acid, maleic acid, fumaric acid, monomers performing a sulfonic acid or phosphonic acid functions, and their salts.

17. A composition according to claim 16, wherein said anionic monomer is acrylic acid.

18. A composition according to claim 1, wherein said chain transfer agent is selected from the group consisting of mercaptanes, malic acid, lactic acid, formic acid, isopropanol and hypophosphites, and mixtures thereof.

\* \* \* \* \*